



US007389638B2

(12) **United States Patent**  
**Weissman et al.**

(10) **Patent No.:** **US 7,389,638 B2**  
(45) **Date of Patent:** **Jun. 24, 2008**

(54) **SULFUR OXIDE/NITROGEN OXIDE TRAP SYSTEM AND METHOD FOR THE PROTECTION OF NITROGEN OXIDE STORAGE REDUCTION CATALYST FROM SULFUR POISONING**

6,482,377 B2 \* 11/2002 Bartley et al. .... 423/213.2  
6,502,391 B1 \* 1/2003 Hirota et al. .... 60/288

(75) Inventors: **Walter Weissman**, Basking Ridge, NJ (US); **El Mekki El Malki**, Princeton, NJ (US)

(Continued)

## FOREIGN PATENT DOCUMENTS

|    |                   |        |
|----|-------------------|--------|
| EP | 1374978 A1        | 1/2004 |
| WO | WO 2004/078644 A1 | 9/2004 |

(73) Assignee: **ExxonMobil Research and Engineering Company**, Annandale, NJ (US)

(\*) Notice: Subject to any disclaimer, the term of this patent is extended or adjusted under 35 U.S.C. 154(b) by 97 days.

(21) Appl. No.: **11/179,372**

(22) Filed: **Jul. 12, 2005**

(65) **Prior Publication Data**

US 2007/0012028 A1 Jan. 18, 2007

(51) **Int. Cl.**  
**F01N 3/00** (2006.01)

(52) **U.S. Cl.** .... **60/286**; 60/275; 60/295

(58) **Field of Classification Search** .... 60/286, 60/275, 295

See application file for complete search history.

(56) **References Cited**

## U.S. PATENT DOCUMENTS

3,948,611 A \* 4/1976 Stawsky .... 422/179  
5,473,890 A \* 12/1995 Takeshima et al. .... 60/285  
5,750,082 A \* 5/1998 Hepburn et al. .... 423/213.5  
5,753,192 A \* 5/1998 Dobson et al. .... 422/177  
6,145,303 A \* 11/2000 Strehlau et al. .... 60/274  
6,272,848 B1 \* 8/2001 Okude et al. .... 60/274  
6,318,075 B1 \* 11/2001 Gunther et al. .... 60/285

Brian West, et al., "Assessing Reductant Chemistry During In-Cylinder Regeneration of Diesel Lean NO<sub>x</sub> Traps" SAE Technical Paper Series #2004-01-3023.

(Continued)

*Primary Examiner*—Thomas Denion*Assistant Examiner*—Loren Edwards(74) *Attorney, Agent, or Firm*—Robert A. Migliorini(57) **ABSTRACT**

The present invention relates to an improved exhaust gas cleaning system and method for a combustion source comprising a hydrogen generation system, a sulfur oxides trap, and a nitrogen storage reduction (NSR) catalyst trap. The improved exhaust gas cleaning system and method of the present invention also provides for a water-gas-shift catalyst between the sulfur oxides trap and the NSR catalyst trap, and a clean-up catalyst downstream of the NSR catalyst trap. The invention provides also a sulfur trap regenerable at moderate temperatures with rich pulses, rather than at high temperatures. The improved exhaust gas cleaning system of the present invention provides for the sulfur released from the sulfur trap to pass through the nitrogen oxide trap with no or little poisoning of NO<sub>x</sub> storage and reduction sites, which significantly improves NSR catalyst trap lifetime and performance to meet future emissions standards. The disclosed exhaust gas cleaning systems are suitable for use in internal combustion engines (e.g., diesel, gasoline, CNG) which operate with lean air/fuel ratios over most of the operating period.

**48 Claims, 24 Drawing Sheets**

## U.S. PATENT DOCUMENTS

|              |      |         |                               |       |           |              |      |         |                          |
|--------------|------|---------|-------------------------------|-------|-----------|--------------|------|---------|--------------------------|
| 6,585,945    | B2 * | 7/2003  | Wu et al.                     | ..... | 423/239.1 | 2004/0170558 | A1   | 9/2004  | Hershkowitz              |
| 6,655,128    | B1 * | 12/2003 | Hei Ma                        | ..... | 60/274    | 2004/0175326 | A1   | 9/2004  | Hershkowitz et al.       |
| 6,691,509    | B2 * | 2/2004  | Hoffman et al.                | ..... | 60/286    | 2004/0180973 | A1   | 9/2004  | Hershkowitz et al.       |
| 6,732,507    | B1 * | 5/2004  | Stanglmaier et al.            | ..... | 60/285    | 2004/0187483 | A1   | 9/2004  | Hershkowitz              |
| 6,745,560    | B2 * | 6/2004  | Stroia et al.                 | ..... | 60/286    | 2004/0191166 | A1   | 9/2004  | Hershkowitz et al.       |
| 6,758,036    | B1 * | 7/2004  | Molinier                      | ..... | 60/286    | 2004/0241505 | A1   | 12/2004 | Hershkowitz et al.       |
| 6,832,473    | B2 * | 12/2004 | Kupe et al.                   | ..... | 60/286    | 2005/0160720 | A1 * | 7/2005  | Elwart et al. .....      |
| 6,933,151    | B2 * | 8/2005  | Bailey et al.                 | ..... | 436/37    | 2005/0178107 | A1 * | 8/2005  | Mital et al. .....       |
| 7,021,048    | B2 * | 4/2006  | Taylor et al.                 | ..... | 60/295    | 2005/0178110 | A1 * | 8/2005  | Mital et al. .....       |
| 7,021,049    | B2 * | 4/2006  | Berris et al.                 | ..... | 60/295    | 2006/0213187 | A1 * | 9/2006  | Kupe et al. .....        |
| 7,082,753    | B2 * | 8/2006  | Dalla Betta et al.            | ..... | 60/286    | 2006/0230748 | A1 * | 10/2006 | Dalla Betta et al. ..... |
| 7,093,428    | B2 * | 8/2006  | LaBarge et al.                | ..... | 60/286    |              |      |         | 60/285                   |
| 7,111,451    | B2 * | 9/2006  | Dou et al.                    | ..... | 60/285    |              |      |         | 60/275                   |
| 7,117,667    | B2 * | 10/2006 | Mital et al.                  | ..... | 60/286    |              |      |         | 60/286                   |
| 2003/0213232 | A1 * | 11/2003 | Brisley et al.                | ..... | 60/285    |              |      |         | 60/286                   |
| 2004/0045285 | A1 * | 3/2004  | Penetrante et al.             | ..... | 60/286    |              |      |         | 60/286                   |
| 2004/0065078 | A1 * | 4/2004  | Schafer-<br>Sindlinger et al. | ..... | 60/295    |              |      |         | 60/286                   |

## OTHER PUBLICATIONS

L. Bromberg et al., "Onboard Plasmatron Generation of Hydrogen rich Gas for Diesel Engine Exhaust Aftertreatment and Other Applications".

\* cited by examiner

**FIGURE 1****FIGURE 2****FIGURE 3**

**FIGURE 4****FIGURE 5**

**FIGURE 6**

**FIGURE 7**

**FIGURE 8**

**FIGURE 9**

**FIGURE 10**

**FIGURE 11**

**FIGURE 12**

**FIGURE 13**

**FIGURE 14**

**FIGURE 15**

**FIGURE 16**

**FIGURE 17**

**FIGURE 18****FIGURE 19**

**FIGURE 20****FIGURE 21**

**FIGURE 22**

**FIGURE 23**

**FIGURE 24**

**FIGURE 25**

**FIGURE 26**

**FIGURE 27**

**FIGURE 28****FIGURE 29**

**FIGURE 30**

**SULFUR OXIDE/NITROGEN OXIDE TRAP  
SYSTEM AND METHOD FOR THE  
PROTECTION OF NITROGEN OXIDE  
STORAGE REDUCTION CATALYST FROM  
SULFUR POISONING**

**FIELD OF THE INVENTION**

The present invention relates to the field of exhaust gas cleaning systems for combustion engines. It more particularly relates to an improved process for operating an exhaust gas treatment unit consisting of a hydrogen rich gas source, a sulfur ( $\text{SO}_x$ ) catalyst trap and a nitrogen oxide ( $\text{NO}_x$ ) storage reduction (NSR) catalyst trap. Still more particularly, the present invention relates to a process based on using a  $\text{H}_2$  gas rich to enable the sulfur released from the sulfur ( $\text{SO}_x$ ) trap to pass through a  $\text{NO}_x$  storage reduction (NSR) catalyst trap with no poisoning of the  $\text{NO}_x$  storage and reduction components.

**BACKGROUND OF THE INVENTION**

In Japan, the  $\text{NO}_x$  storage reduction (NSR) catalyst also known as  $\text{NO}_x$  trap or  $\text{NO}_x$  adsorbent is a demonstrated after treatment technology for control of HC, CO, and  $\text{NO}_x$  on vehicles equipped with lean burn gasoline engines. This catalyst provides two key functions. When the engine operates with a stoichiometric air/fuel ratio, it functions as a standard three-way conversion catalyst. Under lean operating conditions, while CO and HC in the exhaust are combusted, the NSR catalyst trap functions as a trap for  $\text{NO}_x$  ( $\text{NO} + \text{NO}_2$ ). The reaction mechanism of  $\text{NO}_x$  storage and reduction over a NSR catalyst trap are depicted in Equations 1-4. In general, a NSR catalyst trap should exhibit both oxidation and reduction functions. In a lean environment, NO is oxidized to  $\text{NO}_2$  (Equation 1). This reaction is catalyzed by a noble metal (e.g., Pt). Further oxidation of  $\text{NO}_2$  to nitrate, with incorporation of an atomic oxygen occurs. The nitrate is then stored over selected metal components (Equation 2). To ensure continuous and lasting  $\text{NO}_x$  control, the NSR catalyst trap requires periodic regeneration with controlled short, rich pulses, which serve to release (Equation 3) and reduce the stored  $\text{NO}_x$  (Equation 4). Again a Pt group metal is used for  $\text{NO}_x$  release and reduction. Poisoning of the NSR catalyst trap by sulfur oxides takes place in principle in the same way as the storage of nitrogen oxides. The sulfur dioxide emitted by the engine is oxidized to sulfur trioxide on the catalytically active noble metal component (e.g., Pt) of the NSR catalyst trap (Equation 5). Sulfur trioxide ( $\text{SO}_3$ ) reacts with the storage materials (e.g., Ba) in the NSR catalyst trap with the formation of the corresponding sulfates (Equation 6). Because of the low capacity of the trap to hold sulfur before activity falls and of the stability of sulfate poisons, frequent high temperature desulfations under fuel rich conditions are required ( $>650^\circ \text{C}$ ). This stresses the thermal stability of the NSR catalyst trap and ultimately results in a significant fuel penalty as a result of running a fuel rich mixture as required for high temperature desulfations. This correspondingly shortens NSR catalyst trap life.

Equations:



-continued

---

|     |                                                                                               |                                         |
|-----|-----------------------------------------------------------------------------------------------|-----------------------------------------|
| (3) | $\text{M}(\text{NO}_3)_2 + 2\text{CO} = \text{MCO}_3 + \text{NO}_2 + \text{NO} + \text{CO}_2$ | $\text{NO}_x$ release:                  |
| (4) | $\text{NO} + \text{NO}_2 + 3\text{CO} = \text{N}_2 + 3\text{CO}_2$                            | $\text{NO}_x$ reduction to $\text{N}_2$ |
| (5) | $\text{SO}_2 + 1/2 \text{O}_2 = \text{SO}_3$                                                  | $\text{SO}_x$ poisoning Process         |
| (6) | $\text{SO}_3 + \text{MCO}_3 = \text{MSO}_4 + \text{CO}_2$                                     | $\text{SO}_x$ poisoning Process         |

---

In equations 2, 3 and 6, M represents a divalent base metal cation (e.g., Ba). M can also be a monovalent or trivalent metal compound, in which case the equations need to be rebalanced.

One method for decreasing the formation of sulfates that poison the NSR catalyst trap is to provide a  $\text{SO}_x$  trap upstream of the NSR catalyst trap which undergoes a continuous sulfur uptake and release as a function of the air/fuel ratio (A/F ratio). By periodically changing the exhaust gas conditions from lean to rich, the sulfates stored on sulfur trap are decomposed to yield sulfur species, and the nitrates stored on the NSR catalyst trap are reduced to nitrogen. Key requirements are that a substantial fraction of sulfur species released pass through the NSR catalyst trap with no poisoning of the  $\text{NO}_x$  storage (e.g., Ba) and reduction components (e.g., Pt).

EP 0582917 A1 discloses that the poisoning of a storage catalyst with sulfur can be reduced by a sulfur trap inserted into the exhaust gas stream upstream of the storage catalyst. Alkali metals (potassium, sodium, lithium and cesium), alkaline earth metals (barium and calcium), and rare earth metals (lanthanum and yttrium) are disclosed as storage materials for the sulfur trap. The sulfur trap also includes platinum (Pt) as a catalytically active component. However the disadvantage of the embodiments in EP 0582917 A1 is that the sulfur storage capacity is limited, unless an inordinately large trap is provided or the trap is replaced at very frequent intervals. Once the sulfur trap reaches its full storage capacity sulfur oxides contained in the exhaust gas will pass through the sulfur trap and poison the NSR catalyst trap.

U.S. Pat. No. 5,473,890 discloses a  $\text{SO}_x$  trap composition selected from alkali, alkali-earth, and rare earth metals. Pt is also added to this formulation. High temperature regeneration ( $>650^\circ \text{C}$ ) is needed for such a system, which is not a practical solution since this will result in thermal damage to this trap and the NSR unit in the same flow line. U.S. Pat. No. 5,473,890 refers to a  $\text{SO}_x$  trap containing at least one member selected from copper, iron, manganese, nickel sodium, titanium, lithium and titania. In addition Pt is added to the catalyst. Pt containing adsorbents result in significant quantities of  $\text{H}_2\text{S}$  release under rich conditions, which will react with sulfur trap components forming stable metal sulfide leading to only a partial regeneration of  $\text{SO}_x$  trap. The authors did not show any test activity for the system.

U.S. Pat. No. 5,687,565 discloses a very complex oxide composition, selected from alkaline earth oxides (Mg, Ca, Sr, Ba, Zn). In addition Cu and noble metals (Pt, Pd, Ru) were also added. Again such a system is unpractical as a regenerable  $\text{SO}_x$  trap due to the need for  $650^\circ \text{C}$ .+ regeneration and the poisoning effects of  $\text{H}_2\text{S}$  release.

U.S. Pat. No. 5,792,436 discloses  $\text{SO}_x$  traps containing alkaline earth metal oxides selected from Mg, Ca, Sr, Ba in combination with oxides of cerium and a group of elements of atomic numbers from 22 to 29. Pt is also added to the catalysts formulation. Again such a system requires high temperatures to regenerate ( $>650^\circ \text{C}$ ).

EP 1374978 A1 discloses  $\text{SO}_x$  traps containing oxides of copper. The authors indicate that the system can be regenerated at low temperature ( $250$ - $400^\circ \text{C}$ ) depending on the sup-

port. However, the authors did not show any data on the effect of the released sulfur species (e.g., SO<sub>2</sub>) on NSR catalyst trap. As will be discussed later, the released SO<sub>2</sub> at these low temperatures will poison NSR reduction sites under rich conditions.

U.S. Pat. No. 6,145,303 discloses H<sub>2</sub>S formation under rich conditions, and a method to suppress it when the air/fuel ratio is close to stoichiometry. This approach to suppress H<sub>2</sub>S formation translates into a partial and a long regeneration period of the sulfur trap. Moreover, a higher temperature is needed for desulfation, which can also stress the thermal stability of the sulfur trap.

WO 0156686 discloses that the release of sulfur under rich conditions leads to the adsorption of sulfur species on NSR. Also disclosed is that such sulfur adsorption will affect the NSR catalyst trap and a high temperature desulfation procedure of the NSR catalyst trap is needed.

The aforementioned methods for operating an exhaust gas treatment unit consisting of a sulfur trap and a nitrogen oxides storage reduction catalyst have two distinct disadvantages. The first disadvantage is the absence of a procedure to transmit sulfur species through NSR catalyst trap with no poisoning of NO<sub>x</sub> storage and reduction sites. The second disadvantage is that most of the reported sulfur traps contain Pt and are partially regenerated at high temperatures releasing H<sub>2</sub>S as main product. In addition H<sub>2</sub>S may be an issue for future regulation and need to be controlled.

A need exists for an improved process for operating an exhaust gas treatment unit including a sulfur trap and a NSR catalyst trap operated in tandem. The system will ideally have a SO<sub>x</sub> trap regenerable at moderate temperatures (~400-600° C.) by use of a regeneration gas media that can enable the sulfur species released from sulfur trap to pass through the NSR catalyst trap with no poisoning of NO<sub>x</sub> storage and catalytic components.

## SUMMARY OF THE INVENTION

According to the present disclosure, an advantageous exhaust gas cleaning system for a combustion source comprises: a) a H<sub>2</sub> rich gas generator system, b) a sulfur oxides trap, and c) a nitrogen storage reduction (NSR) catalyst trap, wherein the NSR catalyst trap is positioned downstream of the sulfur oxides trap and the H<sub>2</sub> rich gas generator system.

A further aspect of the present disclosure relates to an advantageous method for improving the treatment of exhaust gas comprising the steps of: i) providing a combustion source with an exhaust gas cleaning system comprising a H<sub>2</sub> rich gas generator system, a sulfur oxides storage reduction catalyst trap, and a nitrogen storage reduction (NSR) catalyst trap, wherein the NSR catalyst trap is positioned downstream of the sulfur oxides trap and the H<sub>2</sub> rich gas generator system, and ii) regenerating the sulfur oxides trap and the NSR catalyst trap with the H<sub>2</sub> rich gas and a fuel rich fuel to air engine exhaust gas.

Another aspect of the present disclosure relates to an advantageous exhaust gas cleaning system for a combustion source comprising: a) a H<sub>2</sub> rich gas generator system, b) a nitrogen storage reduction (NSR) catalyst deposited as a contiguous layer on a support material, and c) a sulfur oxides catalyst deposited as a contiguous layer on the NSR catalyst trap, wherein the combined sulfur oxides catalyst and NSR catalyst trap are positioned downstream of the H<sub>2</sub> rich gas generator system.

Another aspect of the present disclosure relates to an advantageous exhaust gas cleaning system for a combustion source comprising: a) a H<sub>2</sub> rich gas generator system, b)

nitrogen storage reduction (NSR) catalyst deposited as a contiguous layer on a support material, c) a water gas shift (WGS) catalyst deposited as a contiguous layer on the NSR catalyst trap, and d) a sulfur oxides catalyst deposited as a contiguous layer on the WGS catalyst, wherein the combined sulfur oxides catalyst, water gas shift catalyst, and NSR catalyst trap are positioned downstream of the H<sub>2</sub> rich gas generator system.

Another aspect of the present disclosure relates to an 10 advantageous method for improving the treatment of exhaust gas comprising the step of providing a combustion source with an exhaust gas cleaning system comprising: a) a H<sub>2</sub> rich gas generator system, b) a sulfur oxides trap, and c) a nitrogen storage reduction (NSR) catalyst trap, wherein the release of 15 sulfur species from the SO<sub>x</sub> trap (mainly as SO<sub>2</sub> with no or little H<sub>2</sub>S) in the presence of moderate amounts of H<sub>2</sub> with no poisoning of NSR sites compared to the release of sulfur species in the presence of hydrocarbons and/or CO.

Another aspect of the present disclosure relates to an 20 advantageous method for improving the treatment of exhaust gas comprising the step of providing a combustion source with an exhaust gas cleaning system comprising: a) a H<sub>2</sub> rich gas generator system, b) a sulfur oxides trap, and c) a nitrogen storage reduction (NSR) catalyst trap, wherein the sulfur 25 regeneration is carried out at a temperature of approximately 400-500° C. each time the NSR catalyst trap is regenerated, such that any H<sub>2</sub>S formed will be trapped by d) a clean-up catalyst trap, downstream of NSR catalyst trap, under rich conditions and released as SO<sub>2</sub> during lean conditions.

Another aspect of the present disclosure relates to an 30 advantageous method for improving the treatment of exhaust gas comprising the step of providing a combustion source with an exhaust gas cleaning system comprising: a) operation of the engine with a rich air/fuel ratio whereby the H<sub>2</sub> is generated directly in the engine exhaust by a tailored late main injection and/or use of a post injection, b) a sulfur oxides trap, and c) a nitrogen storage reduction (NSR) catalyst trap, wherein the sulfur regeneration is carried out at a temperature of approximately 400-600° C. each time the NSR catalyst trap 35 is regenerated, such that any H<sub>2</sub>S formed will be trapped by d) a clean-up H<sub>2</sub>S trap downstream of NSR catalyst trap, under rich conditions and released as SO<sub>2</sub> during lean conditions.

Numerous advantages result from the advantageous 40 exhaust gas cleaning system and method for improving the treatment of exhaust gas disclosed herein and the uses/applications therefore.

For example, in exemplary embodiments of the present disclosure, the disclosed exhaust gas cleaning system comprising a sulfur trap, a hydrogen source, and an NSR catalyst trap exhibits that sulfur released from the sulfur trap subsequently passes through the NSR catalyst trap with no poisoning of NO<sub>x</sub> storage and reduction components.

In a further exemplary embodiment of the present disclosure, the disclosed exhaust gas cleaning system comprising a sulfur trap, a hydrogen source, and an NSR catalyst trap exhibits improved durability of the NSR catalyst trap when positioned downstream of a sulfur trap.

In a further exemplary embodiment of the present disclosure, the disclosed exhaust gas cleaning system comprising a sulfur trap, a hydrogen source, and an NSR catalyst trap exhibits the ability to regenerate both the sulfur trap and the NSR catalyst trap at a temperature below 600° C., which decreases the thermal stress of the catalyst and the fuel penalty.

In a further exemplary embodiment of the present disclosure, the disclosed exhaust gas cleaning system comprising a

sulfur trap, a hydrogen source, and an NSR catalyst trap exhibits improved NSR catalyst lifetime and performance.

In a further exemplary embodiment of the present disclosure, the disclosed exhaust gas cleaning system comprising a sulfur trap, a hydrogen source, and an NSR catalyst trap further includes a shift converter (water gas shift (WGS) catalyst) of improved catalyst composition to efficiently convert carbon monoxide to carbon dioxide and hydrogen without need for special catalyst reconditioning.

In a further exemplary embodiment of the present disclosure, the disclosed exhaust gas cleaning system comprising a sulfur trap, a hydrogen source, and an NSR catalyst trap includes a WGS catalyst of improved composition having increased activity in a shift conversion reactor for converting carbon monoxide to carbon dioxide and hydrogen without need to protect the WGS catalyst from lean conditions.

In a further exemplary embodiment of the present disclosure, the disclosed exhaust gas cleaning system comprising a sulfur trap, a hydrogen source, and an NSR catalyst trap includes a WGS catalyst of improved catalyst composition providing for improved activity and durability over existing catalyst for the water-gas-shift reaction.

These and other advantages, features and attributes of the disclosed exhaust gas cleaning system and method comprising a sulfur trap, a hydrogen source, and an NSR catalyst trap of the present disclosure and their advantageous applications and/or uses will be apparent from the detailed description which follows, particularly when read in conjunction with the figures appended hereto.

#### BRIEF DESCRIPTION OF THE DRAWINGS

To assist those of ordinary skill in the relevant art in making and using the subject matter hereof, reference is made to the appended drawings, wherein:

FIG. 1 depicts an illustrative schematic of a treatment unit for the exhaust gas from an engine according to the present invention. The exhaust gas treatment unit includes a H<sub>2</sub> rich gas generator system (1), a SO<sub>x</sub> trap (2) down-stream of the H<sub>2</sub> generator system (1), and a NSR catalyst trap (3) down-stream of the SO<sub>x</sub> trap (2).

FIG. 2 depicts an illustrative schematic of a treatment unit for the exhaust gas from an engine with the only difference from FIG. 1 being that that the rich gas H<sub>2</sub> generator system (1) is positioned downstream of the SO<sub>x</sub> trap (2) and upstream of the NSR catalyst trap (3).

FIG. 3 depicts an illustrative schematic of an exhaust gas purifying system for an internal combustion engine having a H<sub>2</sub> rich gas generation system (1) and the 3 catalyst systems (sulfur trap (2), a water-gas-shift (WGS) catalyst (2'), and a NSR catalyst trap (3)). The only difference from FIG. 1 is that a WGS catalyst (2') is added upstream of the NSR catalyst trap (3).

FIG. 4 depicts an illustrative schematic of an exhaust gas purifying system for an internal combustion engine, according to the present invention, having a H<sub>2</sub> rich gas generator system (1) and the 3 catalyst systems (sulfur trap (2), a WGS (2'), a NSR catalyst trap (3)), and additionally a clean-up trap/catalyst (4).

FIG. 5 depicts a graphical illustration of the NO<sub>x</sub> reduction at 450° C. over a NSR catalyst trap under simulated rich conditions containing C<sub>3</sub>H<sub>6</sub>/CO in the presence (Feed 2a, Table 1) and absence (Feed 1, Table 1) of sulfur species and with no H<sub>2</sub>.

FIG. 6 depicts a graphical illustration of the effect of SO<sub>2</sub> on NO<sub>x</sub> reduction at 450° C. over a NSR catalyst trap under simulated rich conditions containing H<sub>2</sub> (Feed 2b).

FIG. 7 depicts a graphical illustration of the effect of H<sub>2</sub>S on NO<sub>x</sub> reduction at 300° C. and 450° C. over a NSR catalyst trap under simulated rich conditions containing H<sub>2</sub> (Feed 2b).

FIG. 8 depicts a graphical illustration of the effect of H<sub>2</sub>S on NO<sub>x</sub> reduction at 300° C. over a NSR catalyst trap under simulated rich conditions containing C<sub>3</sub>H<sub>6</sub>/CO (Feed 2a).

FIG. 9 depicts a graphical illustration of NO<sub>x</sub> storage (Feed 4) at 300° C. following 1 cycle poisoning by SO<sub>2</sub> under simulated rich conditions containing C<sub>3</sub>H<sub>6</sub>/CO (Feed 2a) and oxidation (Feed 3) at 450° C. of the adsorbed SO<sub>2</sub>.

FIG. 10 depicts a graphical illustration of NO<sub>x</sub> storage (Feed 4) at 300° C. over a NSR catalyst trap following 1 and 5 cycles poisoning by H<sub>2</sub>S under simulated rich conditions containing C<sub>3</sub>H<sub>6</sub>/CO (Feed 2a) and oxidation (Feed 3) at 450° C. of the adsorbed H<sub>2</sub>S between each cycle.

FIG. 11 depicts a graphical illustration of NO<sub>x</sub> storage (Feed 4) at 300° C. over a NSR catalyst trap following 1 and 5 cycles poisoning by SO<sub>2</sub> under simulated rich conditions containing H<sub>2</sub> (Feed 2b) and oxidation (Feed 3) at 450° C. of the adsorbed H<sub>2</sub>S between each cycle.

FIG. 12. depicts a graphical illustration of NO<sub>x</sub> storage (Feed 4) at 300° C. over a NSR catalyst trap following 1 and 5 cycles poisoning by H<sub>2</sub>S under simulated rich conditions containing H<sub>2</sub> (Feed 2b) and oxidation (Feed 3) at 450° C. of the adsorbed H<sub>2</sub>S between each cycle.

FIG. 13 depicts a graphical illustration of NO<sub>x</sub> storage (Feed 4) at 300° C. over a NSR catalyst trap following 1 and 5 cycles poisoning by H<sub>2</sub>S under simulated rich conditions containing H<sub>2</sub> (Feed 2b) and oxidation (Feed 3) at 300° C. of the adsorbed H<sub>2</sub>S between each cycle.

FIG. 14 depicts a XRD pattern of a pretreated fresh NSR.

FIG. 15 depicts a graphical illustration of SO<sub>2</sub> and H<sub>2</sub>S levels below which bulk solid poisoning of the NSR catalyst trap will not occur as a function of temperature.

FIG. 16 depicts a schematic illustrating sulfur poisoning of Pt and Ba sites in NSR catalyst trap when cycling from rich to lean conditions.

FIG. 17 depicts a graphical illustration of the H<sub>2</sub>/H<sub>2</sub>S ratio needed to avoid PtS formation as a function of temperature during regeneration of the SO<sub>x</sub> catalyst trap.

FIG. 18 depicts a graphical illustration of the first derivative of the weight loss during the reduction of the sulfated metal-containing alumina (Metal=Cu, Fe, Co and Mn).

FIG. 19 depicts a graphical illustration of sulfur species released during the reduction of sulfated Cu/Al<sub>2</sub>O<sub>3</sub> (sulfation at 400° C.).

FIG. 20 depicts a graphical illustration of sulfur species released during the reduction of the sulfated Fe/Al<sub>2</sub>O<sub>3</sub> (sulfation at 400° C.).

FIG. 21 depicts a graphical illustration of sulfur species released during the reduction of the sulfated Co/Al<sub>2</sub>O<sub>3</sub> (sulfation at 400° C.).

FIG. 22 depicts a graphical illustration of sulfur species released during the reduction of the sulfated Mn/Al<sub>2</sub>O<sub>3</sub> (sulfation at 400° C.).

FIG. 23 depicts a graphical illustration of sulfur species released during the reduction of the sulfated Ce/Al<sub>2</sub>O<sub>3</sub> (sulfation at 200° C.).

FIG. 24 depicts a graphical illustration of sulfur species released during the reduction of the sulfated Pt—Fe/Al<sub>2</sub>O<sub>3</sub> (sulfation at 400° C.).

FIG. 25 depicts a graphical illustration of sulfur species released during the thermal decomposition in He of the sulfated Pt—Fe/Al<sub>2</sub>O<sub>3</sub> (sulfation at 400° C.).

FIG. 26 depicts a graphical illustration of sulfur species released during the reduction of a sulfated  $\text{Fe}/\text{Al}_2\text{O}_3$  where an upstream  $\text{Pt}/\text{Al}_2\text{O}_3$  was used during sulfation (sulfation at 400° C.).

FIG. 27 depicts a graphical illustration of sulfur species released during isothermal reduction at 450° C. of a sulfated  $\text{Fe}/\text{Al}_2\text{O}_3$  where an upstream  $\text{Pt}/\text{Al}_2\text{O}_3$  was used during lean sulfation (sulfation at 400° C.).

FIG. 28 depicts a graphical illustration of hydrogen concentration versus temperature and Ce loading on the water gas shift (WGS) reaction over Pt supported  $\text{CeO}_2-\text{ZrO}_2$  for a feed of 4%  $\text{CO}+17\% \text{H}_2\text{O}$  at  $\text{GHSV}=14,683 \text{ h}^{-1}$ .

FIG. 29 depicts a graphical illustration of hydrogen concentration versus temperature and Ce loading on the water gas shift reaction over Pt supported  $\text{CeO}_2-\text{ZrO}_2$  for a feed of 4%  $\text{CO}+17\% \text{H}_2\text{O}$  at  $\text{GHSV}=73,194 \text{ h}^{-1}$ .

FIG. 30 depicts a graphical illustration of hydrogen concentration versus temperature and Ce loading on the water gas shift reaction over Rh supported  $\text{CeO}_2-\text{ZrO}_2$  for a feed of 4%  $\text{CO}+17\% \text{H}_2\text{O}$  at  $\text{GHSV}=14,683 \text{ h}^{-1}$ .

#### DETAILED DESCRIPTION OF THE INVENTION

The present invention relates to an improved exhaust gas treatment system and process for a combustion source. The exhaust gas treatment system and process of the present invention is distinguishable over the prior art in comprising a combination of a sulfur trap (also referred to as a sulfur oxides trap or  $\text{SO}_x$  trap), a hydrogen source (also referred to as a hydrogen generator or generation system), and a nitrogen oxide trap (also referred to as a  $\text{NO}_x$  trap,  $\text{NO}_x$  adsorbent or  $\text{NO}_x$  storage reduction (NSR) catalyst) which in combination advantageously decrease sulfur adsorption, and poisoning of the NSR catalyst trap. More particularly, the present invention relates to an improved system and method for operating an exhaust gas treatment unit including a sulfur trap, a hydrogen source, and a NSR catalyst trap, whereby the process is based on generating  $\text{H}_2$  on-board the vehicle to enable the sulfur released from sulfur trap ( $\text{SO}_2$ ,  $\text{H}_2\text{S}$ ,  $\text{COS}$ ) to pass through the NSR catalyst trap with no poisoning of  $\text{NO}_x$  storage and reduction components. The improved method for operating an exhaust gas treatment unit may also optionally include the addition of a water gas shift catalyst trap, and a clean-up catalyst trap.

The present invention also relates to improvements in an exhaust gas cleaning system, which operates with lean air/fuel ratios over most of the operating period. The exhaust gas treatment unit comprises a nitrogen oxides trap (NSR) catalyst and a sulfur trap located upstream of the nitrogen oxides trap. We discovered that the release of sulfur from a  $\text{SO}_x$  trap as  $\text{SO}_2$  or  $\text{H}_2\text{S}$  in presence of moderate amounts of  $\text{H}_2$  leads to no or a minimal adsorption of sulfur on the NSR catalyst trap when compared to the release of sulfur species in the presence of hydrocarbon (HC) and/or carbon monoxide (CO). This break-through will significantly improve the NSR catalyst trap lifetime and performance. This also permits sulfur regeneration to be carried out at moderate temperature (400-600° C.). In addition, any  $\text{H}_2\text{S}$  formed will be trapped under rich conditions, using a clean-up catalyst trap downstream of the NSR catalyst trap, and released as  $\text{SO}_2$  during lean conditions.

The advantageous effects of incorporating a sulfur trap within the exhaust system are exhibited by monitoring the resulting improved  $\text{NO}_x$  adsorption efficiency. Reference made to the figures that follow show that the  $\text{NO}_x$  storage over the NSR catalyst trap decreases following the release of sulfur species under a simulated rich exhaust containing  $\text{C}_3\text{H}_6/\text{CO}$

(see FIGS. 9, 10). On the other hand,  $\text{NO}_x$  storage was not affected by the release of sulfur species in the presence of  $\text{H}_2$  (see FIGS. 11, 12). In view of this contrast, a further advantage of the present system is that the durability of a NSR catalyst trap when positioned downstream of a sulfur trap can be considerably increased. Another advantage includes the ability to regenerate the sulfur trap and NSR catalyst trap at a temperature below 600° C., which can avoid the thermal stress of the catalyst and the corresponding fuel penalty. A further advantage of the present invention is improved control of hydrogen sulfide, hydrocarbons, and  $\text{NH}_3$  emissions using a clean-up catalyst trap located just downstream of the NSR catalyst trap. These and other advantages will be evident from the detailed disclosure that follows.

The improved exhaust gas treatment unit of the present invention includes a hydrogen source, a sulfur trap (also referred to as a  $\text{SO}_x$  trap or sulfur oxide trap), and a nitrogen oxides trap (NSR catalyst trap). In other exemplary embodiments of the present invention, the improved exhaust gas treatment system additionally includes various combinations of a water-gas-shift catalyst, a clean-up trap, and a diesel particulate collection system. The configuration of these components within the exhaust gas treatment unit may be varied as will be displayed by the embodiments which follow.

The hydrogen source for input to the exhaust gas treatment system may be produced on-board the vehicle by a variety of methods and devices or stored within a refillable reservoir on board the vehicle. An exemplary method of generating  $\text{H}_2$  on-board the vehicle for input to the exhaust gas treatment system is using engine control approaches (in-cylinder injection of excess fuel, or rich combustion). Strategies for engine control employ intake throttling to lower exhaust oxygen concentration, then excess fueling is used to transition rich. For instance Delayed Extended Main (DEM) strategy uses intake throttling to lower Air/Fuel ratio then the main injection duration is extended to achieve rich conditions. On the other hand, a post injection involves adding an injection event after the main injection event to achieve rich operation. Both strategies lead to the conversion of fuel to a mixture of CO and  $\text{H}_2$  (Brian West et al. SAE 2004-01-3023). The CO can further be converted to  $\text{H}_2$  and  $\text{CO}_2$  using a WGS catalyst. Another exemplary method consists on-board plasmatron generation of  $\text{H}_2$  from hydrocarbon fuels as disclosed in U.S. Pat. No. 6,176,078. Other exemplary methods for generating  $\text{H}_2$  utilize catalytic devices. For instance,  $\text{H}_2$  can be produced by steam reforming in which a mixture of deionized water and hydrocarbon fuel are fed to a steam reformer mounted in a combustion chamber as disclosed in U.S. Pat. No. 6,176,078. Further exemplary catalytic devices of generating  $\text{H}_2$  for input to the exhaust gas treatment system include, but are not limited to, autothermal reforming (ATR), pressure swing reforming (as disclosed in U.S. Patent Publication No. 20040170559 and 20041911166), and partial oxidation of hydrocarbon fuels with  $\text{O}_2$  and  $\text{H}_2\text{O}$  (WO patent 01/34950). The catalytic devices always produce a mixture of  $\text{CO}+\text{H}_2$  and a WGS catalyst is needed to convert CO to  $\text{H}_2$  and  $\text{CO}_2$  in presence of water. Another possibility for generating  $\text{H}_2$  is to use an electrolyzer as described in the literature (Heimrich et al. SAE 2000-01-1841). The electrolyzer produces hydrogen from the dissociation of water to hydrogen and oxygen (i.e.,  $\text{H}_2\text{O}=\text{H}_2+\frac{1}{2}\text{O}_2$ ). The produced hydrogen can be injected in the exhaust system or stored under relatively high pressure on-board the vehicle.

Another method of generating additional hydrogen in the exhaust system is to use a water-gas-shift (WGS) catalyst to convert CO (produced by the in-cylinder injection or by catalytic devices) in presence of water to  $\text{CO}_2$  and  $\text{H}_2$  by using

suitable elements and supports for such. The overall reaction is as follows:  $\text{CO} + \text{H}_2\text{O} = \text{CO}_2 + \text{H}_2$  whereby  $\Delta H = -41.2 \text{ kJ/mol}$ , and  $\Delta G = -28.6 \text{ kJ/mol}$ . A commonly used catalyst for the WGS reaction is  $\text{CuO-ZnO-Al}_2\text{O}_3$  based catalyst (U.S. Pat. No. 4,308,176). However, the performance of the catalyst to effect carbon monoxide conversion and the hydrogen yield gradually decrease during normal operations due to deactivation of the catalyst. In addition because of the sensitivity of this catalyst to air and condensed water, there is a reason not to use them for an automotive fuel processing devices.

Metal-promoted ceria catalysts have been tested as water-gas-shift catalysts (T. Shido et al, *J. Catal.* 141 (1994) 105; J. T. Kummer, *J. Phys. Chem.* 90 (1986) 4747). The combination of ceria and platinum provide a catalyst that is more oxygen tolerant than earlier known catalysts. Moreover, ceria is known to play a crucial role in automotive, three-way, emissions-control because of its oxygen-storage capacity (H. C. Yao et al. *J. Catal.* 86 (1984) 254). Deactivation of the oxygen storage capacity of ceria by high temperatures in automotive applications is well known, and it is necessary to stabilize the reducibility of ceria for that application by mixing it with zirconia (Shelef et al. "Catalysis by Ceria and related Materials", Imperial College press, London 2002, p. 243).

The improved catalyst composition for the WGS of the present invention used in the shift converter comprises a noble metal catalyst having a promoting support. The support comprises a mixed metal oxide of at least cerium oxide and zirconium oxide. The zirconia increases the resistance of ceria to sintering, thereby improving the durability of the catalyst composition. Additionally, alumina may be added to the catalyst composition to improve its suitability for wash-coating onto a monolithic substrate. An exemplary combination of catalyst element and support material of the present invention for a WGS catalyst is Pt supported on ceria, Pt supported on ceria-zirconia, Rh supported on ceria, Rh supported on ceria-zirconia, or combinations thereof.

The present invention further includes sulfur ( $\text{SO}_x$ ) trap upstream of WGS catalyst to protect the WGS and the NSR trap from sulfur poisoning under lean conditions. The release of sulfur species will occur in the temperatures range of 400-600° C. to avoid any adsorption of sulfur species on NSR. The sulfur ( $\text{SO}_x$ ) trap may be prepared by using known techniques for the preparation of vehicle exhaust gas catalysts. The sulfur trap includes a catalyst composition suitable for adsorbing  $\text{SO}_x$  as metal sulfate under lean (oxidative) conditions and desorbing accumulated sulfate as  $\text{SO}_2$  under rich (reducing) conditions. The composition of the sulfur trap is further designed to prevent sulfur poisoning of after treatment devices, and especially the NSR catalyst trap. The sulfur oxide trap elements are selected based on their ability to release sulfur at low temperatures (<600° C.) under rich exhaust conditions.

Suitable sulfur ( $\text{SO}_x$ ) traps are selected from oxides of copper, iron, cobalt, manganese, tin, ceria, zirconia, lithium, titania and combinations thereof. The aforementioned  $\text{SO}_x$  adsorbent materials may be used as mixed metal oxides or supported on alumina, stabilized gamma alumina, silica, MCM-41, zeolites, titania, and titania-zirconia. For example, the sulfur oxides trap may include an oxide of the structure  $\text{Fe}/\text{x}$  oxide wherein x is selected from the group consisting of  $\text{Al}_2\text{O}_3$ ,  $\text{SiO}_2$ ,  $\text{ZrO}_2$ ,  $\text{CeO}_2-\text{ZrO}_2$ ,  $\text{TiO}_2-\text{Al}_2\text{O}_3$ , MCM-41, and Zeolites. Another suitable method for improving  $\text{SO}_x$  adsorption at low temperature is to use an upstream Pt oxidation catalyst.

The nitrogen storage reduction (NSR) catalyst (also referred to as nitrogen oxide trap,  $\text{NO}_x$  trap,  $\text{NO}_x$  adsorbent)

may be selected from the noble metals, including, but not limited to Pt, Pd, Rh, and combinations thereof, and a porous carrier or substrate carrying the noble metals, including, but not limited to alumina, MCM-41, zeolites, titania, and titania-zirconia. The NSR catalyst trap may further include alkali metals and/or alkaline earth metals, for example, Li, K, Cs, Mg, Ca, Sr, Ba and combinations of the alkali metals and alkaline earth metals. The NSR catalyst trap may also include ceria, zirconia, titania, lanthanum and other similar materials, which are typically employed in a three-way catalyst. Other NSR formulations described in the literature may also be used.

In a further preferred embodiment, the exhaust system according to the invention includes a clean-up catalyst trap downstream of the NSR. This is particularly useful with  $\text{SO}_x$  traps wherein during regeneration produce  $\text{H}_2\text{S}$ , which has an unpleasant smell. In order to combat this, the clean-up catalyst trap comprises a component for suppressing  $\text{H}_2\text{S}$ , for example oxides of one or more of nickel, manganese, cobalt and iron. Such components are useful at least because of their ability to trap hydrogen sulfide under rich or stoichiometric conditions and, at lean conditions, to promote the oxidation of hydrogen sulfide to sulfur dioxide. In an alternative embodiment, the clean-up catalyst can also be configured so as to contend with HC slip past the oxidation catalyst of the invention, which can occur where there is insufficient oxygen in the gas stream to oxidize the HC to  $\text{H}_2\text{O}$  and  $\text{CO}_2$ . In this case, the clean-up catalyst includes an oxygen storage component with catalytic activity, such as ceria and/or Pt group metals (PGM). The clean-up catalyst trap may also contain a  $\text{NH}_3$  trap which may form during regeneration of the NSR catalyst trap. The  $\text{NH}_3$  trap preferably includes zeolites such as ZSM-5, Beta, MCM-68, or metal containing zeolites, wherein the metal can be selected from Fe, Co, and Cu. The trapped  $\text{NH}_3$  can then react with  $\text{NO}_x$  to form  $\text{N}_2$  under lean conditions. If necessary, air can be injected upstream of the clean-up catalyst during rich regeneration of the  $\text{SO}_x$  trap.

All the catalysts systems (catalytic  $\text{H}_2$  generation,  $\text{SO}_x$  trap, NSR, WGS and clean-up catalyst) described above may be provided on a separate substrate such as a flow-through honeycomb monolith. The monolith may be metal or ceramic, where ceramic it can be cordierite, although alumina, mullite, silicon carbide, zirconia are alternatives. Manufacture of coated substrate may be carried out by methods known to one skilled in the art.

A catalyzed Diesel Particulate Filter (DPF) system may be optionally positioned (for a diesel engine) upstream of the sulfur trap to remove particulate matter from the engine exhaust source. The DPF system is particularly advantageous when combusting diesel fuels. A variety of DPF and filter configurations are available in the market today (Summers et al. *Applied Catalysis B: 10 (1996) 139-156*). The most common design of DPF is the wall-flow monolith, which consists of many small parallel ceramic channels running axially through the part (Diesel particulate traps, wall-flow monoliths, Diesel Technology Guide at [www.dieselnet.com](http://www.dieselnet.com)). Adjacent channels are alternatively plugged at each end in order to force the diesel exhaust gases through the porous substrate walls, which act as a mechanical filter. As the particulate (soot) load increases and the need for regeneration increases. The regeneration requires the oxidation of the collected particulate matter. Pt may be added to DPF to enhance such oxidation.

The above systems may be organized into various configurations to yield improved exhaust gas treatment systems. The various configurations include, but are not limited to, a series arrangement of the systems, a layered arrangement of the

## 11

systems, and a combination of a series and layered arrangement of the systems. The various configurations of the exhaust gas treatment system will be demonstrated by the exemplary embodiments which follow.

FIG. 1 depicts an exemplary embodiment of the present invention for an improved exhaust gas treatment unit comprising a combustion engine exhaust source, a hydrogen generator system (1), a SO<sub>x</sub> trap (2) downstream of the H<sub>2</sub> generator system (1), and a NSR catalyst trap (3) downstream of the SO<sub>x</sub> trap (2). During the lean operation of the engine, SO<sub>2</sub> is oxidized to SO<sub>3</sub> which is trapped as sulfate on sulfur trap (2) components. During the rich operation of the engine and at a temperature of 450° C., the sulfates are decomposed, and the released sulfur species pass through NSR catalyst trap (3) in the presence of H<sub>2</sub> (1). The quantities of sulfur oxides contained in the exhaust gas from an internal combustion engine are much smaller than the quantities of nitrogen oxides, and therefore, it is not necessary to also remove sulfur from the sulfur oxide trap each time the nitrogen oxides are released from the storage catalyst. The period of the cycle for releasing nitrogen oxides from the NSR catalyst trap is about one minute, whereas the period for releasing from the sulfur trap is several hours. The exemplary embodiment of FIG. 1 with the hydrogen generated upstream of the sulfur trap is suitable when the hydrogen source originates from the combustion engine.

FIG. 2 depicts an alternative exemplary embodiment of a treatment unit for an exhaust gas according to the present invention comprising a combustion engine exhaust source, a SO<sub>x</sub> trap (2), a hydrogen generator system (1) downstream of the SO<sub>x</sub> trap (2), and a NSR catalyst trap (3) downstream of the hydrogen generator system (1). The only difference from FIG. 1 is the position of the H<sub>2</sub> generator system (1) being positioned downstream of the SO<sub>x</sub> trap (2) and upstream of the NSR catalyst trap (3). The exemplary embodiment of FIG. 2 with the hydrogen injected between the sulfur trap and the NSR catalyst trap is particularly suitable when the hydrogen source originates from a source other than the combustion engine.

FIG. 3 depicts an alternative exemplary embodiment of an exhaust gas purifying system for an internal combustion engine according to the present invention including a H<sub>2</sub> generation system (1) and 3 catalyst systems (sulfur trap (2), a water-gas-shift (WGS) catalyst (2'), and a NSR catalyst trap (3)). The H<sub>2</sub> generation system (1) is positioned downstream of the engine exhaust source and upstream of the sulfur trap (2). A WGS catalyst (2') is positioned downstream of the sulfur trap (2) and upstream of a NSR catalyst trap (3). The only difference from FIG. 1 is that a WGS catalyst (2') is added upstream of the NSR catalyst trap (3).

FIG. 4 depicts a further exemplary embodiment of an exhaust gas purifying system for an internal combustion engine, according to the present invention, having a H<sub>2</sub> generator system (1), 3 catalyst systems (sulfur trap (2), a WGS catalyst (2'), a NSR catalyst trap (3)), and additionally a clean-up catalyst (4). The H<sub>2</sub> generation system (1) is positioned downstream of the engine exhaust source and upstream of the sulfur trap (2). A WGS catalyst (2') is positioned downstream of the sulfur trap (2) and upstream of a NSR catalyst trap (3). A clean-up catalyst (4) is then positioned downstream of the NSR catalyst trap (3). The only difference from FIG. 3 is the addition of a clean-up catalyst trap (4) downstream of the NSR catalyst trap (3).

The preceding exemplary embodiments may further include a particulate removal system downstream of the engine exhaust source and upstream of both the hydrogen generation system (1) and the sulfur trap (2). The particulate

## 12

removal system is particularly advantageous when a diffusion flame type combustion is utilized, for example as in current day diesel engines, since this leads to soot formation.

The catalyst comprising the exhaust gas treatment system 5 may be alternatively configured in a layered arrangement by forming layers of one or more of the various catalysts (SO<sub>x</sub>, WGS, NSR catalysts) on top of one another. For example, the NSR catalyst trap is deposited as a contiguous layer on a suitable support material, and then the sulfur oxide catalyst is 10 deposited as a contiguous layer on top of the NSR catalyst trap layer. In an alternative exemplary embodiment, the NSR catalyst trap is deposited as a contiguous layer on a suitable support material, the WGS catalyst deposited as a contiguous layer on top of the NSR catalyst trap layer, and then the sulfur oxide catalyst deposited as a contiguous layer on top of the WGS catalyst layer. In these layered catalyst configurations, the exhaust gas diffuses first through the outer sulfur oxide catalyst layer, followed by the WGS catalyst layer, and finally 15 the through NSR catalyst trap layer. These exemplary layered catalyst configurations are coupled with an upstream hydrogen generation source. In addition, these exemplary layered catalyst configurations may be optionally configured with an upstream particulate removal system, and a downstream clean-up catalyst trap.

Applicants have attempted to disclose all embodiments 20 and applications of the disclosed subject matter that could be reasonably foreseen. However, there may be unforeseeable, insubstantial modifications that remain as equivalents. While the present invention has been described in conjunction with specific, exemplary embodiments thereof, it is evident that 25 many alterations, modifications, and variations will be apparent to those skilled in the art in light of the foregoing description without departing from the spirit or scope of the present disclosure. Accordingly, the present disclosure is intended to embrace all such alterations, modifications, and variations of the above detailed description.

The following examples from feasibility studies to pass 30 sulfur species (SO<sub>2</sub>, H<sub>2</sub>S) through the NSR catalyst trap during sulfur trap regeneration illustrate the present invention and the advantages thereto without limiting the scope thereof.

## Test Methods

In terms of catalyst preparation, the NSR catalyst trap used 45 for these studies was supplied in washcoated monolith from a commercial source. The washcoat composition contains NO<sub>x</sub> reduction sites (Pt/Rh), a storage compound (Ba), support (γ-Al<sub>2</sub>O<sub>3</sub>), and other promoters selected from ceria, titania, zirconia and lanthanum. The catalyst was pretreated at 450° C. for 15 minutes under simulated rich exhaust before testing 50 (see Table 1, Feed 1).

The monolithic NSR core (0.75 in length×0.5 in diameter) is placed in a quartz reactor on top of a piece of quartz wool with several inches of crushed fused quartz added as a preheat 55 zone. The quartz reactor is heated by a furnace. The temperature is controlled by a type-K thermocouple located inside a quartz thermowell inside the narrowed exit portion of the reactor located below the monolithic core. The activity tests were conducted in a flow reactor system by using different gas mixtures as depicted in Table 1. A FTIR and a Mass Spectrometer (MS) were used to analyze the gas phase effluents (e.g., NO, NO<sub>2</sub>, H<sub>2</sub>S, SO<sub>2</sub>, N<sub>2</sub>O, NH<sub>3</sub>, CO, CO<sub>2</sub>, etc.). Two rich gas mixtures were considered for sulfur species adsorption 60 on the catalyst. The first gas consists of 90 ppm SO<sub>2</sub> (or H<sub>2</sub>S), 2000 ppm C<sub>3</sub>H<sub>6</sub>, 1000 ppm CO, 11% CO<sub>2</sub>, 6% H<sub>2</sub>O in He (Table 1, Feed 2a). The second gas consists of 90 ppm SO<sub>2</sub> (or H<sub>2</sub>S), 1% H<sub>2</sub>, 11% CO<sub>2</sub>, 6% H<sub>2</sub>O in He (Table 1, Feed 2b).

The sulfur species adsorbed while flowing a rich gas mixture were then oxidized under a lean gas mixture (Table 1, Feed 3) before measuring  $\text{NO}_x$  storage capacity of the catalyst. Tests for  $\text{NO}_x$  storage capacity were done at 300°C. flowing a lean gas mixture containing NO (Table 1, Feed 4) over both fresh and sulfur-poisoned NSR catalyst. After  $\text{NO}_x$  adsorption as nitrate, a regeneration step is used to decompose the nitrate using a rich gas mixture (Feed 2a or Feed 2b) free of  $\text{SO}_2$  or  $\text{H}_2\text{S}$ .

TABLE 1

| Rich-lean gas mixtures used at the laboratory test experiments |                                     |                                        |         |                                                                |                                             |         |
|----------------------------------------------------------------|-------------------------------------|----------------------------------------|---------|----------------------------------------------------------------|---------------------------------------------|---------|
| Components in the feed                                         | Pre-treatment under rich conditions | Sulfur poisoning under rich conditions |         | Oxidation of the adsorbed sulfur species under lean conditions | $\text{NO}_x$ storage under lean conditions |         |
|                                                                |                                     | Feed 1                                 | Feed 2a | Feed 2b                                                        | Feed 3                                      | Feed 4  |
| $\text{SO}_2$ or $\text{H}_2\text{S}$ (ppm)                    | 0                                   | 90                                     | 90      | 0                                                              | 0                                           | 0       |
| NO (ppm)                                                       | 250                                 | 250                                    | 250     | 250                                                            | 250                                         | 250     |
| $\text{C}_3\text{H}_6$ (ppm)                                   | 2000                                | 2000                                   | 0       | 2000                                                           | 0                                           | 0       |
| CO (ppm)                                                       | 1000                                | 1000                                   | 0       | 1000                                                           | 0                                           | 0       |
| $\text{H}_2$ (%)                                               | 0                                   | 0                                      | 1       | 0                                                              | 0                                           | 0       |
| $\text{CO}_2$ (%)                                              | 11                                  | 11                                     | 11      | 11                                                             | 11                                          | 11      |
| $\text{O}_2$ (%)                                               | 0                                   | 0                                      | 0       | 7                                                              | 7                                           | 7       |
| $\text{H}_2\text{O}$ (%)                                       | 6                                   | 6                                      | 6       | 6                                                              | 0                                           | 0       |
| He                                                             | balance                             | balance                                | balance | Balance                                                        | balance                                     | balance |

The total flow rate was 3000 cc/min, which corresponds to a space velocity of 49,727 h<sup>-1</sup> (@ STP). The temperature was varied from 300 to 600°C.

FTIR. The spectrometer used was a Nicolet 670. A liquid nitrogen cooled MCT (Hg/Cd/Te) IR detector was used to provide a high-signal-to-noise ratio. Because of the narrow natural linewidth of the small gas molecules studied, we operated at a resolution of 0.5 cm<sup>-1</sup>. At this resolution, one scan requires 1.5 seconds. Background spectra were collected daily, with the cell filled with flowing dry He. Two gas cells with a path length of 2 and 10 m, equipped with ZnSe windows were used. The cell was heated to a temperature of 165°C.

Mass spectrometer. A quadrupole MS (Pfeifer vacuum system) was used for sulfur species analysis

XRD. X-ray powder diffraction patterns were recorded on a Siemens D500 diffractometer using Cu K $\alpha$  radiation.

Thermodynamic calculations. The thermodynamic calculations were performed using the commercial software HSC Chemistry.

## EXAMPLES

### Example 1

#### Effect of $\text{SO}_2$ and $\text{H}_2\text{S}$ on $\text{NO}_x$ Reduction Efficiency at 450°C.

The interaction of sulfur species with noble metal sites (e.g., Pt and/or Rh) can directly be determined by looking to  $\text{NO}_x$  reduction under rich conditions. Any poisoning of noble metal sites will translate into a decrease in  $\text{NO}_x$  conversion. FIG. 5 depicts a graphical illustration of the effect of trapped  $\text{SO}_2$  and  $\text{H}_2\text{S}$  on  $\text{NO}_x$  reduction at 450°C. under a simulating rich exhaust containing  $\text{C}_3\text{H}_6$ /CO (Feed 2a). As can be seen in FIG. 5, 100%  $\text{NO}_x$  conversion is achieved without sulfur. Upon addition of sulfur species ( $\text{SO}_2$  or  $\text{H}_2\text{S}$ ),  $\text{NO}_x$  conver-

sion decreases as a function of exposure time. For instance, after 15 minutes of exposure to  $\text{SO}_2$ ,  $\text{NO}_x$  conversion decreases by about 20%. This decrease reached 50% in the presence of  $\text{H}_2\text{S}$ , indicating that sulfur poisoning of noble metal sites is more severe with  $\text{H}_2\text{S}$  than with  $\text{SO}_2$ .  $\text{NO}_x$  conversion stabilizes at around 40%, which indicates only a partial poisoning of the noble metal sites. FIG. 6 depicts a graphical illustration of the effect of  $\text{SO}_2$  on  $\text{NO}_x$  reduction at 450°C. under a simulating rich exhaust containing 1%  $\text{H}_2$  (Feed 2b). As depicted in the figure, 100%  $\text{NO}_x$  conversion is obtained, which shows no poisoning of noble metal sites. FIG. 7 depicts a graphical illustration of the effect of  $\text{H}_2\text{S}$  on  $\text{NO}_x$  reduction at 300°C. and at 450°C. under rich gas mixtures containing  $\text{H}_2$  (Feed 2b). As can be seen, at 300°C.  $\text{NO}_x$  conversion decreases, but stabilizes at around 50%, which again indicates the poisoning of only a fraction of the noble metal sites. On the other hand at 450°C., 100%  $\text{NO}_x$  conversion is obtained, showing no poisoning of noble metal sites. FIG. 8 depicts a graphical illustration of the effect of  $\text{H}_2\text{S}$  on  $\text{NO}_x$  reduction at 300°C. under rich gas mixtures containing  $\text{C}_3\text{H}_6$ /CO (Feed 2a). As can be seen, a complete poisoning of metal sites (Pt and Rh) when the NSR catalyst trap is exposed to rich gas mixtures containing CO/ $\text{C}_3\text{H}_6$  and in presence of  $\text{H}_2\text{S}$  at 300°C. Indeed,  $\text{NO}_x$  conversion was completely lost after a 10 minute exposure to  $\text{H}_2\text{S}$ , and even after removal of  $\text{H}_2\text{S}$ , the  $\text{NO}_x$  conversion was not restored indicating irreversible poisoning of noble metal sites. However, after addition of 500 ppm oxygen to the rich mixture (Feed 2a), full recovery of  $\text{NO}_x$  conversion is observed indicating noble metal sites regenerated.

The decrease in  $\text{NO}_x$  conversion in the presence of sulfur species (FIG. 5) is attributed to the formation of metal sulfide (e.g., PtS) due to  $\text{H}_2\text{S}$  and  $\text{SO}_2$  dissociation over noble metal sites. The fact that under the conditions used  $\text{NO}_x$  conversion stabilizes to around 40-50% in the presence of sulfur species (FIGS. 5, 7) indicates that a limited portion of noble metal sites are poisoned by sulfur. Based on published literature, we attribute the decrease in  $\text{NO}_x$  conversion to the poisoning of Pt sites, but not of Rh sites. Indeed, early laboratory studies of Pt and Rh in three-way catalysts (TWC) showed sulfur inhibition of catalytic activity to be dependent upon both catalyst composition and the operating conditions (W. B. Pierson et al., *SAE paper*, 790942 (1979). W. B. Williamson et al., *Env. Sci. Tech.*, 14 (1980) 319. J. C. Summers and K. Baron, *J. Catal.*, 57 (1979) 266. G. C. Joy et al. *SAE paper*, 790943 (1979)). It was found that  $\text{SO}_2$  severely inhibited  $\text{NO}_x$  conversion and ammonia formation over Pt under fuel rich operating conditions, but had minimal effect on the  $\text{NO}_x$  performance of Rh catalysts. The sulfur inhibition was found to be much lower under stoichiometric conditions. It was also found that  $\text{NO}_x$  reduction over Rh is higher than over Pt, both in the presence and absence of  $\text{SO}_2$ . The difference in performance between Rh and Pt is more pronounced when  $\text{SO}_2$  is present due to the greater sulfur inhibition of the Pt catalyst (J. C. Summers and K. Baron, *J. Catal.*, 57 (1979) 266). In the presence of CO,  $\text{SO}_2$  was not adsorbed on the Rh catalyst, but coadsorption of CO and  $\text{SO}_2$  was observed on the Pt catalyst (H. S. Gandhi et al., *SAE paper* 780606 (1978)). These literature results reveal a stronger interaction of sulfur species with Pt than with Rh. Another interesting observation is that the addition of small amount of  $\text{O}_2$  to rich exhaust leads to full recovery of  $\text{NO}_x$  reduction (FIG. 8) indicating that sulfide species can be removed from the noble metal surface, apparently achieved by the reverse of reaction 3 and formation of  $\text{SO}_3$  as shown in reaction:



15

One issue with adding oxygen to avoid noble metal poisoning is that the oxidation of the adsorbed sulfide species leads to the formation of  $\text{SO}_3$  which can then poison  $\text{NO}_x$  storage components (e.g., Ba sites).

## Example 2

$\text{NO}_x$  ( $\text{NO}+\text{NO}_2$ ) Adsorption Under Lean Conditions  
(Feed 3) at 300° C. after Oxidation of Adsorbed  
Sulfur Species

In order to exhibit the extent that  $\text{NO}_x$  storage sites (e.g., Ba) are poisoned by the trapped sulfur species, we have evaluated  $\text{NO}_x$  storage efficiency at 300° C. under lean conditions (Table 1, Feed 4) for a fresh NSR trap and after different cycles of sulfur-poisoning. Each cycle of poisoning consists of treating Pt-containing  $\text{NO}_x$  trap at 300 or 450° C. with a rich gas feed containing  $\text{SO}_2$  or  $\text{H}_2\text{S}$  (Table 1, Feed 2a or 2b) for 30 minutes followed by oxidation under lean conditions (Table 1, Feed 3) for 15 minutes. Any poisoning of  $\text{NO}_x$  storage sites (e.g., Ba) by sulfur translates into a decrease in  $\text{NO}_x$  storage efficiency. The  $\text{NO}_x$  storage was evaluated using Feed 4 (Table 1).

FIG. 9 depicts a graphical illustration of  $\text{NO}_x$  storage efficiency (Feed 3) at 300° C. following 1 cycle poisoning by  $\text{SO}_2$  under simulated rich conditions containing  $\text{C}_3\text{H}_6/\text{CO}$  (Feed 2a) and oxidation (Feed 3) at 450° C. of the adsorbed  $\text{SO}_2$ . FIG. 10 depicts a graphical illustration of  $\text{NO}_x$  storage efficiency (Feed 3) at 300° C. of NSR catalyst trap following 1 and 5 cycles poisoning by  $\text{H}_2\text{S}$  under simulated rich conditions containing  $\text{C}_3\text{H}_6/\text{CO}$  (Feed 2a) and oxidation (Feed 3) at 450° C. of the adsorbed  $\text{H}_2\text{S}$  between each cycles. FIG. 11 depicts a graphical illustration of  $\text{NO}_x$  storage efficiency (Feed 4) at 300° C. following 1 and 5 cycles poisoning by  $\text{SO}_2$  under simulated rich conditions containing  $\text{H}_2$  (Feed 2b) and oxidation at 450° C. (Feed 3) of the adsorbed  $\text{SO}_2$  between each cycle. FIG. 12 depicts a graphical illustration of  $\text{NO}_x$  storage efficiency (Feed 4) at 300° C. following 1 and 5 cycle poisoning by  $\text{H}_2\text{S}$  under simulated rich conditions containing  $\text{H}_2$  (Feed 2b) and oxidation at 450° C. (Feed 3) of the adsorbed  $\text{H}_2\text{S}$  between each cycle. FIG. 13 depicts a graphical illustration of  $\text{NO}_x$  storage efficiency (Feed 4) at 300° C. following 1 and 5 cycle poisoning by  $\text{H}_2\text{S}$  under simulated rich conditions containing  $\text{H}_2$  (Feed 2b) and oxidation at 450° C. (Feed 3) of the adsorbed  $\text{H}_2\text{S}$  between each cycle.

FIGS. 8-13 depict the  $\text{NO}_x$  storage efficiency under lean conditions (Feed 4) of the poisoned NSR catalyst trap either by  $\text{SO}_2$  (FIGS. 9, 11) or  $\text{H}_2\text{S}$  (FIGS. 10, 12, 13). The oxidation with Feed 3 of the adsorbed sulfur species during rich conditions containing  $\text{C}_3\text{H}_6/\text{CO}$  (Feed 2a) affects  $\text{NO}_x$  storage components (e.g., Ba sites) after 1 cycle poisoning by a 12 and 20% decrease in  $\text{NO}_x$  storage capacity with respectively  $\text{SO}_2$  (FIG. 9) and  $\text{H}_2\text{S}$  (FIGS. 10, 13). The  $\text{NO}_x$  storage efficiency continues to decrease after 5 cycle poisoning with  $\text{H}_2\text{S}$  (FIGS. 10, 13) and a loss of 40-50% is observed in line with  $\text{NO}_x$  storage components poisoning (e.g., formation of  $\text{BaSO}_4$  after oxidation of adsorbed sulfur species). On the other hand, the  $\text{NO}_x$  storage efficiency is not affected when NSR catalyst trap was exposed to sulfur species in the presence of  $\text{H}_2$  at 450° C. (FIG. 11 and FIG. 12). In presence of  $\text{SO}_2$  (FIG. 11), the  $\text{NO}_x$  storage capacity even after 5 cycle poisoning is comparable to fresh catalyst. In the presence of  $\text{H}_2\text{S}$  (FIG. 12), no difference between fresh and poisoned catalyst after the first 10 minutes and only minor change is observed after that with the respect to the experimental error. Even in presence of  $\text{H}_2$ , the temperature needs to be controlled to avoid any storage efficiency loss. Indeed,  $\text{NO}_x$  storage capacity

16

decreases by 20 to 50% when the NSR catalyst trap was exposed to  $\text{H}_2\text{S}$  in presence of  $\text{H}_2$  at 300° C. (FIG. 13).

## Example 3

Understanding Sulfur Interaction with  $\text{NO}_x$  Storage  
Sites (e.g., Ba) and  $\text{NO}_x$  Reduction Sites (e.g. Pt)

To understand the interaction of sulfur species with barium sites, it is important to determine at what conditions (rich/lean) barium sites are poisoned by sulfur. Under rich conditions, barium sites exist mainly as barium carbonate as indicated by XRD (FIG. 14). Thermodynamic calculation (FIG. 15) shows that 90 ppm of  $\text{SO}_2$  or  $\text{H}_2\text{S}$  species can pass through barium carbonate at 450° C. without forming  $\text{BaSO}_3$  or  $\text{BaS}$ . Hence, it can be concluded that under rich gas mixtures and a temperature of 450° C., no adsorption of sulfur species on barium sites occurs. It is important to understand why barium carbonate sites are poisoned by the trapped sulfur species under lean conditions. There is a correlation between the sulfur poisoning of noble metal sites under rich conditions and barium sites under lean conditions. Indeed, any decrease in  $\text{NO}_x$  reduction efficiency in the presence of sulfur species under rich conditions (see FIGS. 5, 7, 8) over a NSR catalyst trap leads to a decrease in  $\text{NO}_x$  storage capacity under lean conditions (see FIGS. 6, 9, 10, 13). On the other hand, when 100%  $\text{NO}_x$  reduction is observed under rich conditions (FIGS. 6, 7), no  $\text{NO}_x$  storage loss under lean conditions is observed (FIGS. 11, 12). A simple scheme to explain the poisoning of barium and Pt sites is presented in FIG. 16. Under rich conditions, ( $\text{C}_3\text{H}_6/\text{CO}$ ) sulfur species interact with Pt sites forming  $\text{PtS}$  and then when switching to lean conditions, the adsorbed sulfide are oxidized to  $\text{SO}_3$ , which then reacts with the barium carbonate forming  $\text{BaSO}_4$ . To avoid the  $\text{PtS}$  formation,  $\text{H}_2$  is needed to shift the equilibrium of the reaction of  $\text{Pt}+\text{H}_2\text{S}=\text{PtS}+\text{H}_2$ . To shift the equilibrium to the right, it is important to control the temperature and  $\text{H}_2$  concentration. As typified in FIG. 17,  $\text{H}_2/\text{H}_2\text{S}$  is needed to avoid  $\text{PtS}$  formation. For instance at 450° C., the  $\text{H}_2/\text{H}_2\text{S}$  needs to be higher than 50. The  $\text{H}_2/\text{H}_2\text{S}$  ratio decreases with increasing temperature.

In summary, this study shows that under simulated rich conditions (presence of  $\text{C}_3\text{H}_6$  and  $\text{CO}$ , no oxygen), sulfur species were trapped on the NSR catalyst trap at temperatures from 300° C. to 450° C. Such adsorption leads to a poisoning of noble metal sites as evidenced by a decrease of  $\text{NO}_x$  reduction. When switching to lean conditions, the trapped sulfur species poison barium sites as evidenced by a decrease in  $\text{NO}_x$  storage capacity. Under these conditions, a sulfur trap upstream of the commercial NSR catalyst trap is not feasible and bypassing the NSR is needed if such conditions will be used. On the other hand, this study shows that sulfur adsorption under rich conditions can be minimized/or eliminated by releasing the sulfur species  $\text{SO}_2/\text{H}_2\text{S}$  in the presence of  $\text{H}_2$  at a temperature of 450° C. At this temperature,  $\text{BaSO}_3/\text{BaS}$  formation is unfavorable and it appears that  $\text{H}_2$  prevents the adsorption of sulfur on Pt sites. In addition, the comparison of  $\text{NO}_x$  storage capacity between fresh and sulfur poisoned NSR catalyst trap shows similar trapping efficiency in line with no sulfur poisoning of barium sites. The implication of this finding is that the development of a sulfur trap upstream of the commercial NSR catalyst trap is feasible if  $\text{H}_2$  can be provided during sulfur trap regeneration. To take advantage of these findings, strategies need to be developed to generate  $\text{H}_2$  on-board the vehicle. In addition a regenerable  $\text{SO}_x$  trap in the temperature range of 400-600° C. is needed to avoid sulfur

adsorption by the NSR catalyst trap and also to limit the high temperature desulfation (>650° C.) of the catalyst.

Examples 4 to 9

Sulfur Trap Preparation, Sulfation, and Regeneration Preparation

Sulfur Trap Preparation:

The support used in this work was a commercial  $\text{Al}_2\text{O}_3$  (with different surface area). The  $\text{Al}_2\text{O}_3$  support was first calcined at 550° C. for 4 hours. The dried  $\text{Al}_2\text{O}_3$  was then impregnated with metal salts solution selected from Fe, Cu, Mn, Ce, Co, Pt and other components. The metal contents was varied from 0.5 to 30 wt % against 100 wt %  $\text{Al}_2\text{O}_3$  support, respectively. Other supports such as  $\text{SiO}_2$ ,  $\text{ZrO}_2$ ,  $\text{CeO}_2$ — $\text{ZrO}_2$  and ZSM-5 were also used.

$\text{Cu}/\text{Al}_2\text{O}_3$  catalyst (Example 4) was accomplished by the incipient method technique. This technique involves the addition of an aqueous solution of copper salt to a dry  $\text{Al}_2\text{O}_3$  carrier until reaching incipient wetness. The concentration of the aqueous copper solution was adjusted to the desired Cu loading. As a typical example 1.8301 grams of copper nitrate hemipentahydrate ( $\text{Cu}(\text{NO}_3)_2 \cdot 2.5\text{H}_2\text{O}$ ) was dissolved in 5.2 ml of deionized water. To this solution was added 5 grams of the dried  $\text{Al}_2\text{O}_3$ . The as prepared solid was mixed then dried in a vacuum oven at 80° C. and calcined in air at 550° C. for 4 hours. The final sulfur trap contained copper in an amount of 10 wt % per 100 wt % of  $\text{Al}_2\text{O}_3$ . The copper is present in the calcined sample as copper oxide.

$\text{Mn}/\text{Al}_2\text{O}_3$  catalyst (Example 5) was prepared in the same way as in Example 4. Differently from Example 4, the  $\text{Al}_2\text{O}_3$  was impregnated with manganese nitrate hydrate. The final sulfur trap contained manganese in an amount of 10 wt % per 100 wt % of  $\text{Al}_2\text{O}_3$ . The manganese is present in the calcined sample as manganese oxide.

$\text{Co}/\text{Al}_2\text{O}_3$  catalyst (Example 6) was prepared in the same way as in Example 4. Differently from Example 4, the  $\text{Al}_2\text{O}_3$  was impregnated with cobalt (II) acetate tetrahydrate. The final sulfur trap contained cobalt in an amount of 10 wt % per 100 wt % of  $\text{Al}_2\text{O}_3$ . The cobalt is present in the calcined sample as cobalt oxide.

$\text{Fe}/\text{Al}_2\text{O}_3$  catalyst (Example 7) was prepared in the same way as in Example 4. Differently from Example 4, the  $\text{Al}_2\text{O}_3$  was impregnated with iron (III) nitrate nonahydrate. The final sulfur trap contained iron in amount of 10 wt % per 100 wt % of  $\text{Al}_2\text{O}_3$ . The iron is present in the calcined sample as iron oxide.

$\text{Ce}/\text{Al}_2\text{O}_3$  catalyst (Example 8) was prepared in the same way as in Example 4. Differently from Example 4, the  $\text{Al}_2\text{O}_3$  was impregnated with cerium (III) nitrate hexahydrate. The final sulfur trap contained Cerium in an amount of 20 wt % per 100 wt % of  $\text{Al}_2\text{O}_3$ . The cerium is present in the calcined sample as cerium oxide.

$\text{Pt—Fe}/\text{Al}_2\text{O}_3$  catalyst (Example 9) was prepared as follows: the  $\text{Al}_2\text{O}_3$  support was impregnated with an aqueous solution of platinum (II) tetra amine nitrate, dried at 80° C., then calcined in He 450° C. for 1 hour. The final sample contains 2 wt % Pt. Following these steps, the dried  $\text{Pt}/\text{Al}_2\text{O}_3$  was then impregnated by renewed immersion in aqueous solution of iron (III) nitrate nonahydrate, dried at 80° C. and calcined at 550° C. for 4 hours in air. The calcined sample contained 2 wt % Pt and 10 wt % Fe.

An oxidation  $\text{Pt}/\text{Al}_2\text{O}_3$  catalyst (Example 10) was prepared following a similar procedure as Example 9. This oxidation catalyst was used upstream system of sulfur traps described in Examples 4 through 7.

Sulfation:

The sulfur trap catalysts from examples 4 through 9 were tested in a bench flow reactor with a simulated lean exhaust gases containing  $\text{SO}_2$ . The simulated lean exhaust gas contained 30 ppm  $\text{SO}_2$ , 5%  $\text{H}_2\text{O}$ , 5%  $\text{CO}_2$  and 10%  $\text{O}_2$  at a gas hourly space velocity of 60.000/hr. The higher than typical sulfur dioxide concentration, 30 ppm, is utilized to accelerate the sulfation. Typically 0.5 grams of catalysts (14-25 mesh size) from examples 4 through 9 was loaded in a quartz reactor then temperature heating was increased from 25° C. to 550° C. at 10° C./min under 10%  $\text{O}_2$ ; holding sample for 1 hour at 550° C.; cooling to the desired temperature in the range of 200 to 500° C. At the desired temperature the simulated lean exhaust feed containing  $\text{SO}_2$  was then passed through the catalyst for 20 hrs and then the catalyst was purged with 10%  $\text{O}_2$  in helium for 30 min. For comparison, the  $\text{Pt}/\text{Al}_2\text{O}_3$  oxidation catalyst (Example 10) was placed upstream of the sulfur traps of Examples 4 through 8. The layered catalysts were then sulfated at the same conditions (see above).

Regeneration:

The sulfated sulfur traps (see sulfation procedure above) were regenerated in a 10%  $\text{H}_2$  in He. Also, a thermal decomposition of the metal sulfate was performed in He. Approximately 20 mg of the sulfated sample was placed on the TGA balance (TGA/SDTA 851, Mettler Toledo, Inc.) and the gas feed ( $\text{H}_2$  in He or He) was passed through the sample while the temperature was increased from 30° C. to 800° C. at a temperature ramp rate of 10° C./min. The sulfur species released from the sulfated sample were analyzed by on-line Mass Spectrometer (Pfeiffer Vacuum System). FIG. 18 shows the first derivative of the weight loss (as determined by TGA) during reduction of metal sulfate (e.g., sulfation at 400° C.). As can be seen, different maxima of the weight loss are observed for different metal sulfate. For instance, the maximum temperature weight loss is observed at 300° C. for  $\text{Cu}/\text{Al}_2\text{O}_3$ , at 460° C. for  $\text{Fe}/\text{Al}_2\text{O}_3$ , at 520° C. for  $\text{Co}/\text{Al}_2\text{O}_3$ , and at 620° C. for  $\text{Mn}/\text{Al}_2\text{O}_3$ . The MS signal of the released sulfur species ( $\text{SO}_2$ : m/e=64 and  $\text{H}_2\text{S}$ : m/e=34) corresponding to this weight loss under  $\text{H}_2$  are shown in FIGS. 19-22. As can be seen, the  $\text{SO}_2$  was the major product of sulfur reduction. For  $\text{Cu}/\text{Al}_2\text{O}_3$  sample, one can see two peaks of  $\text{SO}_2$  release at 300° C. and 350° C. Also, the  $\text{H}_2\text{S}$  desorption peak is observed at high temperature (>450° C.) (FIG. 19). For  $\text{Fe}/\text{Al}_2\text{O}_3$ , a single  $\text{SO}_2$  desorption peak is observed at 460° C. and a complete desorption below 500° C. (FIG. 20). For  $\text{Co}/\text{Al}_2\text{O}_3$ , a single desorption peak for  $\text{SO}_2$  is observed at max temperature of 520° C. (FIG. 21). In addition,  $\text{H}_2\text{S}$  was also observed at high temperature (>600° C.). For  $\text{Mn}/\text{Al}_2\text{O}_3$ , the maximum  $\text{SO}_2$  desorption peak can be seen at 625° C. with a complete desorption at temperature of 650° C. (FIG. 22).

The regeneration of sulfated  $\text{Ce}/\text{Al}_2\text{O}_3$  (sulfation at 200° C.) in 10%  $\text{H}_2$  in He leads to two desorption peaks of  $\text{SO}_2$  (at 580° C.) and  $\text{H}_2\text{S}$  (at 630° C.) as shown in FIG. 23. With controlling the temperature below 600° C. it will be possible to avoid  $\text{H}_2\text{S}$  emissions.

The regeneration of the sulfated  $\text{Pt—Fe}/\text{Al}_2\text{O}_3$  (sulfation at 400° C.) under 10%  $\text{H}_2$  in He shows no desorption of sulfur species at temperatures below 600° C. and only  $\text{H}_2\text{S}$  is observed at temperature higher than 650° C. (FIG. 24). On the other hand, when  $\text{H}_2$  is replaced with He, the sulfate decomposition from the sulfated sample occurs in the temperature range of 400-650° C. (FIG. 25). The sulfur is released mainly as  $\text{SO}_2$ . These results clearly indicate that under  $\text{H}_2$  flow, the sulfur is retained on the catalyst. In the presence of Pt, the

19

sulfate is reduced to  $H_2S$  which then can react with iron to form stable iron sulfide (e.g.,  $FeS$ ). In conclusion, it is important to keep sulfur traps free from Pt. One way to take advantage of the Pt is to use it as an upstream oxidation catalyst with a downstream Pt free sulfur trap (layered catalysts) selected from Examples 4 through 7. In this case the oxidation of  $SO_2$  to  $SO_3$  occurs upstream of sulfur trap without influencing the desorption of sulfur species from sulfur traps. As typical examples, FIGS. 26-27 show sulfur species release from the sulfated  $Fe/Al_2O_3$  catalyst (sulfation done with an upstream  $Pt/Al_2O_3$  from Example 10). Only one desorption peak is observed at maximum temperature of  $460^\circ C$ . (FIG. 26). Also when an isothermal temperature was used ( $450^\circ C$ . a complete desorption of sulfur as  $SO_2$  occurs and no sulfur desorption is observed when the temperature was increased from  $450^\circ C$ . to  $700^\circ C$ ., indicative of complete sulfur desorption from iron at  $450^\circ C$ . (FIG. 27).

In summary,  $Cu/Alumina$  system shows desorption peaks for sulfur as  $SO_2$  at or below  $300$ - $350^\circ C$ . However, at this temperature the  $SO_2$  will poison NSR catalyst trap sites (see FIGS. 5, 8 and 7). Also,  $Mn/Al_2O_3$  shows higher temperature desorption peak ( $>600^\circ C$ .) which is not practical as a regenerable sulfur trap.  $Co/Al_2O_3$  and  $Fe/Al_2O_3$  are the preferred sulfur trap candidates as the sulfur can be released in the temperature range of  $400$ - $600^\circ C$ . Also, it is very important to mention a complete isothermal regeneration of sulfated  $Fe/Al_2O_3$  (e.g.,  $450^\circ C$ .) producing only  $SO_2$  but no  $H_2S$  which can present significant advantage of our invention. At this temperature, the sulfur species can pass through the NSR catalyst trap in presence of the desired amount of  $H_2$  without any poisoning of the active sites. Also, it is important to keep the sulfur trap free from noble metal (e.g., Pt). The Pt group metal can be used in an upstream position to help low temperature adsorption (below  $300^\circ C$ .) by enhancing  $SO_2$  oxidation to  $SO_3$ . Another possibility for low temperature adsorption is to use ceria-supported catalyst or stabilized ceria-zirconia down-stream of the Pt free sulfur trap. A typical optimized sulfur trap will have an upstream Pt-containing oxidation catalyst (e.g.,  $Pt/Al_2O_3$  or Pt-containing DPF system), Pt free  $SO_x$  trap (e.g.,  $Fe/Al_2O_3$ ) and a downstream ceria-containing sample.

For exhaust automobile application these catalysts can be provided on a separate substrate such as a flow-through honeycomb monolith. The monolith can be metal or ceramic, where ceramic it can be cordierite, although alumina, mullite, silicon carbide, zirconia are alternatives. Manufacture of coated substrate can be carried out by methods known to the skilled in the art and no further explanation will be given here.

## Examples 11-12

Water Gas Shift Catalyst Preparation and Pretreatment for  $CeO_2-ZrO_2$  Supports

2.6%  $CeO_2-ZrO_2$  sample (Example 11). Five hundred grams of  $ZrOCl_2 \cdot 8H_2O$  and fourteen grams of  $Ce(SO_4)_2$  were dissolved while stirring in 3.0 liters of distilled water. Another solution containing 260 grams of concentrated  $NH_4OH$  and 3.0 liters of distilled water was prepared. These two solutions were combined at the rate of 50 ml/min using a nozzle for mixing. The pH of the final composite was adjusted to approximately 8 by the addition of concentrated ammonium hydroxide. This slurry was then put in polypropylene bottles and placed in a steambox ( $100^\circ C$ .) for 72 hours. The product formed was recovered by filtration, washed with excess water, and stored as a filtercake. The filtercake was dried overnight at  $100^\circ C$ . Thereafter a portion of the dried filter-

20

cake was calcined at  $700^\circ C$ . for a total of 3 hours in flowing air and then allowed to cool. The cerium content was 2.6%. Sample nomenclature was 2.6%  $CeO_2-ZrO_2$ .

17.65%  $CeO_2-ZrO_2$  sample (Example 12). Five hundred grams of  $ZrOCl_2 \cdot 8H_2O$  and one hundred and forty grams of  $Ce(SO_4)_2$  were dissolved while stirring in 3.0 liters of distilled water. Another solution containing 260 grams of concentrated  $NH_4OH$  and 3.0 liters of distilled water was prepared. These two solutions were combined at the rate of 50 ml/min using nozzle mixing. The pH of the final composite was adjusted to approximately 8 by the addition of concentrated ammonium hydroxide. This slurry was then put in polypropylene bottles and placed in a steambox ( $100^\circ C$ .) for 72 hours. The product formed was recovered by filtration, washed with excess water, and stored as a filtercake. The filtercake was dried overnight at  $100^\circ C$ . Thereafter a portion of the filtercake was calcined at  $700^\circ C$ . for a total of 3 hours in flowing air. The cerium content was 17.6%. Sample nomenclature was 17.65%  $CeO_2-ZrO_2$ .

Testing of the WGS was done using stainless steel laboratory microreactors. The catalyst (25-30 mesh size) was loaded in the reactor and then reduced in 4%  $H_2$  in helium at  $400^\circ C$ . for 2 hours before the WGS reaction. Water was then fed to the evaporator (at  $120^\circ C$ .). Then mixed in the evaporator with the carbon monoxide (CO) and nitrogen ( $N_2$ ) feed gas. The gas mixture passed into the fixed bed laboratory microreactor via heated lines ( $110^\circ C$ .). Gaseous products ( $CO_2, H_2$ ) from the reactor were quantified using the thermal conductivity detector (TCD) of a Hewlett Packard 6890 gas chromatograph. The gas mixture consisting of the following:  $CO=4\%$ ,  $H_2O=17\%$  and a total flow rate such that the  $GHSV=14,638\ h^{-1}$ .

$CeO_2-ZrO_2$  catalysts were inactive for the WGS reaction in the temperature range of  $150$ - $450^\circ C$ .

## Examples 13 and 14

Water Gas Shift Catalyst Preparation for  $CeO_2-ZrO_2$  Pt Supported on  $CeO_2-ZrO_2$ 

2.6%  $CeO_2-ZrO_2$  and 17.6%  $CeO_2-ZrO_2$  supports prepared in Example 4 and 6 were loaded with Pt as follows: 51 mg of the tetraammineplatinum (II) chloride hydrate was dissolved in 30 ml of water, and then 3 g of the  $CeO_2-ZrO_2$  were added. The mixture was stirred for 4 hours. The pH of the solution was 2.41 with the 2.6%  $CeO_2-ZrO_2$  while this value reached 2.83 when 17.6%  $CeO_2-ZrO_2$  was used. The excess solution was removed by heating at  $90^\circ C$ . while stirring. After drying in an oven overnight the solids were calcined at  $400^\circ C$ . for 4 hours in air. The Pt loading in the samples was 1 wt %.

The Pt/2.6%  $CeO_2-ZrO_2$  (Example 13) and Pt/17.6%  $CeO_2-ZrO_2$  (Example 14) were reduced at  $400^\circ C$ . in 4%  $H_2$  in He then tested for their WGS performance at different temperatures and a total flow rate such that the  $GHSV=14,638\ h^{-1}$  (FIG. 28), or at a  $GHSV$  of 73,  $194\ h^{-1}$  (FIG. 29). As can be seen, from FIGS. 28 and 29 the catalysts are active at a broad temperature window. At the temperature below  $350^\circ C$ ., Pt/2.6%  $CeO_2-ZrO_2$  shows a high  $H_2$  production than the Pt/17.6%  $CeO_2-ZrO_2$  indicating the importance of cerium loading in controlling the acidity of the support and Pt dispersion. Increasing the  $GHSV$  lead to a decrease in the WGS activity in both catalysts. At the temperature of interest to our application (e.g.,  $450^\circ C$ .), the  $H_2$  produced is in the range 2.3-2.6% with a CO conversion in the range 60-70%.

Water Gas Shift Catalyst Preparation and Testing of Rh Supported on CeO<sub>2</sub>—ZrO<sub>2</sub> Catalysts

2.6% CeO<sub>2</sub>—ZrO<sub>2</sub> and 17.6% CeO<sub>2</sub>—ZrO<sub>2</sub> supports prepared in Examples 11-12 were loaded with Rh as follows: 37.5 mg of Rhodium (III) trichloride were dissolved in 30 ml water then 3 g of the CeO<sub>2</sub>—ZrO<sub>2</sub> were added. The mixture was stirred for 4 hours. The pH of the solution was 2.25 with the 2.6% CeO<sub>2</sub>—ZrO<sub>2</sub> (Example 11), and this value reached 2.58 when 17.6% CeO<sub>2</sub>—ZrO<sub>2</sub> (Example 12) was used. The excess solution was removed by heating at 90° C. while stirring. After drying at 80° C. in an oven overnight, the solid was calcined at 400° C. for 4 hours in air. The Rh loading in the samples was 0.5 wt %.

The as prepared catalysts were reduced in 4% H<sub>2</sub> in He at 400° C. then tested for their WGS performance in a gas mixture consisting of: CO=4%, 17% H<sub>2</sub>O and a total flow rate such that the GHSV=14,638 h<sup>-1</sup> (FIG. 30). As can be seen, both catalysts show comparable activity with a maximum H<sub>2</sub> concentration at around 2.5% at 450° C. and with a CO conversion of 70%.

The WGS catalyst can be provided on a separate substrate such as a flow-through honeycomb monolith. The monolith can be metal or ceramic, where ceramic it can be cordierite, although alumina, mullite, silicon carbide, zirconia are alternatives. Manufacture of coated substrate can be carried out by methods known to the skilled in the art and no further explanation will be given here. In other embodiment the WGS components can be included in NSR catalyst trap formulation. Also, the WGS components can be layered with the NSR components on the same monolith.

What is claimed is:

1. An exhaust gas cleaning system for a combustion source comprising:
  - a) a H<sub>2</sub> rich gas generator system,
  - b) a sulfur oxides trap, and
  - c) a nitrogen storage reduction (NSR) catalyst trap,
 wherein the NSR catalyst trap is positioned downstream of the sulfur oxides trap and the H<sub>2</sub> rich gas generator system, wherein the sulfur oxides trap releases sulfur atom species during regeneration under a rich fuel to air ratio condition to the downstream NSR catalyst trap, wherein the NSR catalyst trap is at a temperature of from about 400 to about 600° C. in the presence of H<sub>2</sub> from the H<sub>2</sub> rich gas generator system, and at an atomic ratio of H<sub>2</sub> to the released sulfur atom species of greater than or equal to about 65 during regeneration of the sulfur oxides trap, and
- wherein the sulfur atom species released by the sulfur oxides trap pass through the NSR catalyst trap with no poisoning of the NO<sub>x</sub> storage and NO<sub>x</sub> reduction components.
2. The exhaust gas cleaning system of claim 1, wherein the H<sub>2</sub> rich gas generator system is positioned upstream of the sulfur oxides trap.
3. The exhaust gas cleaning system of claim 1, wherein the H<sub>2</sub> rich gas generator system is positioned downstream of the sulfur oxides trap.
4. The exhaust gas cleaning system of claim 1, wherein the H<sub>2</sub> rich gas generator system is selected from the group consisting of an engine management system using in-cylinder fuel injection, an on-board refillable hydrogen storage container, an on-board plasmatron generator, an on-board steam

reformer, an on-board auto thermal reformer, an on-board pressure swing reformer, and an on-board water electrolysis system.

5. The exhaust gas cleaning system of claim 4 further comprising a water gas shift catalyst positioned downstream of the sulfur oxides trap and upstream of the NSR catalyst trap.

10 6. The exhaust gas cleaning system of claim 5, wherein the water gas shift catalyst comprises Pt supported on ceria-zirconia, Pt supported on ceria, Rh supported on ceria-zirconia, Rh supported on ceria, or combinations thereof.

7. The exhaust gas cleaning system of claim 4 further comprising a water gas shift catalyst within the NSR catalyst trap.

15 8. The exhaust gas cleaning system of claim 7, wherein the water gas shift catalyst comprises Pt supported on ceria-zirconia, Pt supported on ceria, Rh supported on ceria-zirconia, Rh supported on ceria, or combinations thereof.

20 9. The exhaust gas cleaning system of claim 1, wherein the sulfur oxides trap comprises an oxide selected from the group consisting of copper, iron, manganese, cobalt, ceria, zirconia, tin, titanium, lanthanum, lithium, bismuth, and combinations thereof.

25 10. The exhaust gas cleaning system of claim 9, wherein the sulfur oxides trap adsorbs SO<sub>x</sub> as a metal sulfate at a temperature from about 200° C. to about 550° C. under a lean fuel to air ratio condition.

30 11. The exhaust gas cleaning system of claim 10, wherein the sulfur oxides trap releases atomic sulfur species at a temperature from about 300 to about 600° C. under a rich fuel to air ratio condition and in the absence of or presence of H<sub>2</sub> from the H<sub>2</sub> rich gas generator system.

35 12. The exhaust gas cleaning system of claim 11, wherein the sulfur oxides trap releases atomic sulfur species at a temperature from about 400° C. to about 550° C. under a rich fuel to air ratio condition.

40 13. The exhaust gas cleaning system of claim 9, wherein the sulfur oxides trap further comprises a support material selected from the group consisting of alumina, stabilized gamma alumina, MCM-41, zeolites, silica titania, titania-zirconia, and combinations thereof.

45 14. The exhaust gas cleaning system of claim 13, wherein the sulfur oxides trap adsorbs SO<sub>x</sub> as metal sulfate at a temperature from about 200° C. to about 550° C. under a lean fuel to air ratio condition.

50 15. The exhaust gas cleaning system of claim 14, wherein the sulfur oxides trap releases atomic sulfur species at a temperature from about 300° C. to about 600° C. under a rich fuel to air ratio condition and in absence of or presence of H<sub>2</sub> from the H<sub>2</sub> rich gas generator system.

55 16. The exhaust gas cleaning system of claim 15, wherein the sulfur oxides trap releases atomic sulfur species at a temperature from about 400° C. to about 550° C.

17. The exhaust gas cleaning system of claim 1 further comprising a platinum (Pt) group metal containing oxidation catalyst, a non-Pt group metal containing diesel particulate filter, or a Pt group metal containing diesel particulate filter positioned upstream of the sulfur oxide trap, wherein the platinum group metal is selected from the group consisting of Pt, Rh, Pd, and combinations thereof.

18. The exhaust gas cleaning system of claim 17, wherein the diesel particulate filter is washcoated with sulfur oxides trap components.

60 19. The exhaust gas cleaning system of claim 1, wherein the NSR catalyst trap comprises an alkali metal, an alkaline earth metal, or combinations thereof.

23

20. The exhaust gas cleaning system of claim 19, wherein the NSR catalyst trap further comprises a platinum group metal selected from the group consisting of Pt, Rh, Pd, and combinations thereof.

21. The exhaust gas cleaning system of claim 19, wherein the NSR catalyst trap further comprises ceria, zirconia, titania, iron, cobalt, manganese, nickel, lanthanum, alumina, or combinations thereof.

22. The exhaust gas cleaning system of claim 1 wherein the NSR catalyst trap is at a temperature of from about 400 to about 550° C.

23. The exhaust gas cleaning system of claim 1 wherein the NSR catalyst trap is at a temperature of from about 400 to about 500° C.

24. The exhaust gas cleaning system of claim 1 wherein the NSR catalyst trap is at a temperature of from about 400 to about 450° C.

25. The exhaust gas cleaning system of claim 1 wherein the NSR catalyst trap is at a temperature of from about 550 to about 600° C. in the presence of H<sub>2</sub> from the H<sub>2</sub> rich gas generator system, and at an atomic ratio of H<sub>2</sub> to the released sulfur atom species of greater than or equal to about 13.

26. The exhaust gas cleaning system of claim 1 wherein the NSR catalyst trap is at a temperature of from about 500 to about 600° C. in the presence of H<sub>2</sub> from the H<sub>2</sub> rich gas generator system, and at an atomic ratio of H<sub>2</sub> to the released sulfur atom species of greater than or equal to about 18.

27. The exhaust gas cleaning system of claim 1 wherein the NSR catalyst trap is at a temperature of from about 450 to about 600° C. in the presence of H<sub>2</sub> from the H<sub>2</sub> rich gas generator system, and at an atomic ratio of H<sub>2</sub> to the released sulfur atom species of greater than or equal to about 42.

28. A method for improving the treatment of exhaust gas comprising the steps of:

i) providing a combustion source with an exhaust gas cleaning system comprising:

a) a H<sub>2</sub> rich gas generator system,  
b) a sulfur oxides trap, and

c) a nitrogen storage reduction (NSR) catalyst trap,

wherein the NSR catalyst trap is positioned downstream of the sulfur oxides trap and the H<sub>2</sub> rich gas generator system,

ii) regenerating the sulfur oxides trap through the release of sulfur atom species under a rich fuel to air ratio condition to the downstream NSR catalyst trap, and

iii) maintaining the NSR catalyst trap at a temperature of from about 400 to about 600° C. in the presence of H<sub>2</sub> from the H<sub>2</sub> rich gas generator system at an atomic ratio of H<sub>2</sub> to the released sulfur atom species of greater than or equal to about 65 during regeneration of the sulfur oxides trap

wherein the sulfur atom species released by the sulfur oxides trap pass through the NSR catalyst trap with no poisoning of the NO<sub>x</sub> storage and NO<sub>x</sub> reduction components.

29. The method for improving the treatment of exhaust gas of claim 28 further comprising a clean-up catalyst trap positioned downstream of the NSR catalyst trap.

30. The method for improving the treatment of exhaust gas of claim 29, wherein the clean-up catalyst trap adsorbs hydrogen sulfide in a rich fuel to air ratio condition and releases SO<sub>2</sub> in a lean fuel to air ratio condition.

31. The method for improving the treatment of exhaust gas of claim 30, wherein the clean-up catalyst trap comprises a base metal oxide selected from the group consisting of iron oxide, nickel oxide, manganese oxide, cobalt oxide, and combinations thereof.

24

32. The method for improving the treatment of exhaust gas of claim 31, wherein the base metal oxide is supported on a material selected from the group consisting of alumina, stabilized gamma alumina, MCM-41, zeolites, titania, titania-zirconia, and combinations thereof.

33. The method for improving the treatment of exhaust gas of claim 29, wherein the clean-up catalyst trap comprises components for HC/CO oxidation selected from the group consisting of ceria, a platinum group metal, and combinations thereof.

34. The method for improving the treatment of exhaust gas of claim 33, wherein the components for HC/CO oxidation are supported on a material selected from the group consisting of alumina, stabilized gamma alumina, MCM-41, zeolites, titania, titania-zirconia, and combinations thereof.

35. The method for improving the treatment of exhaust gas of claim 29, wherein the clean-up catalyst comprises components for NH<sub>3</sub> trapping selected from the group consisting of acidic metal oxides, zeolites, and metal-containing zeolites.

36. The method for improving the treatment of exhaust gas of claim 35, wherein the acidic metal oxides are selected from the group consisting of tungsten-zirconia, sulfated zirconia, sulfated ceria-zirconia, phosphated zirconia, and phosphated ceria zirconia.

37. The method for improving the treatment of exhaust gas of claim 35, wherein the zeolites are selected from the group consisting of ZSM-5, Beta, MCM-68, Faujasite, and MCM-41.

38. The method for improving the treatment of exhaust gas of claim 35, wherein the metal-containing zeolites comprise a metal selected from the group consisting of copper, iron, cobalt and silver.

39. The method for improving the treatment of exhaust gas of claim 28, wherein a catalyzed diesel particulate filter is positioned upstream of the sulfur oxides trap.

40. The method for improving the treatment of exhaust gas of claim 28, wherein the step of regenerating the sulfur trap catalyst trap and the NSR catalyst trap with a fuel rich air/fuel ratio is in presence of a low concentration of H<sub>2</sub> at a temperature of about 450° C. to about 550° C.

41. The method of claim 28 comprising the step of: iii) maintaining the NSR catalyst trap at a temperature of from about 400 to about 550° C.

42. The method of claim 28 comprising the step of: iii) maintaining the NSR catalyst trap at a temperature of from about 400 to about 500° C.

43. The method of claim 28 comprising the step of: iii) maintaining the NSR catalyst trap at a temperature of from about 400 to about 450° C.

44. The method of claim 28 comprising the step of: iii) maintaining the NSR catalyst trap at a temperature of from about 550 to about 600° C. in the presence of H<sub>2</sub> from the H<sub>2</sub> rich gas generator system at an atomic ratio of H<sub>2</sub> to the released sulfur atom species of greater than or equal to about 13.

45. The method of claim 28 comprising the step of: iii) maintaining the NSR catalyst trap at a temperature of from about 500 to about 600° C. in the presence of H<sub>2</sub> from the H<sub>2</sub> rich gas generator system at an atomic ratio of H<sub>2</sub> to the released sulfur atom species of greater than or equal to about 18.

46. The method of claim 28 comprising the step of: iii) maintaining the NSR catalyst trap at a temperature of from about 450 to about 600° C. in the presence of H<sub>2</sub> from the H<sub>2</sub> rich gas generator system at an atomic ratio of H<sub>2</sub> to the released sulfur atom species of greater than or equal to about 42.

**25**

**47.** An exhaust gas cleaning system for a combustion source comprising:

- a) a H<sub>2</sub> rich gas generator system,
- b) a nitrogen storage reduction (NSR) catalyst deposited as a contiguous layer on a support material, and
- c) a sulfur oxides catalyst deposited as a contiguous layer on the NSR catalyst,

wherein the combined sulfur oxides catalyst and NSR catalyst trap are positioned downstream of the H<sub>2</sub> rich gas generator systems,

wherein the sulfur oxides catalyst releases sulfur atom species during regeneration under a rich fuel to air ratio condition to the NSR catalyst,

wherein the NSR catalyst is at a temperature of from about 400 to about 600° C. in the presence of H<sub>2</sub> from the H<sub>2</sub> rich gas generator system, and at an atomic ratio of H<sub>2</sub> to the released sulfur atom species of greater than or equal to about 65 during regeneration of the sulfur oxides trap, and

wherein the sulfur atom species released by the sulfur oxides trap pass through the NSR catalyst trap with no poisoning of the NO<sub>x</sub> storage and NO<sub>x</sub> reduction components.

**48.** An exhaust gas cleaning system for a combustion source comprising:

**26**

- a) a H<sub>2</sub> rich gas generator system,
- b) a nitrogen storage reduction (NSR) catalyst deposited as a contiguous layer on a support material,
- c) a water gas shift (WGS) catalyst deposited as a contiguous layer on the NSR catalyst trap, and
- d) a sulfur oxides catalyst deposited as a contiguous layer on the water gas shift catalyst,

wherein the combined sulfur oxides catalyst, WGS catalyst, and NSR catalyst trap are positioned downstream of the H<sub>2</sub> rich gas generator system,

wherein the sulfur oxides catalyst releases sulfur atom species during regeneration under a rich fuel to air ratio condition to the NSR catalyst,

wherein the NSR catalyst is at a temperature of from about 400 to about 600° C. in the presence of H<sub>2</sub> from the H<sub>2</sub> rich gas generator system, and at an atomic ratio of H<sub>2</sub> to the released sulfur atom species of greater than or equal to about 65 during regeneration of the sulfur oxides trap, and

wherein the sulfur atom species released by the sulfur oxides trap pass through the NSR catalyst trap with no poisoning of the NO<sub>x</sub> storage and NO<sub>x</sub> reduction components.

\* \* \* \* \*